



US007105285B2

(12) **United States Patent**  
Ninomiya et al.

(10) **Patent No.:** US 7,105,285 B2  
(45) **Date of Patent:** Sep. 12, 2006

(54) **SILVER HALIDE COLOR PHOTOSENSITIVE MATERIAL**

(75) Inventors: **Toshitaka Ninomiya**, Minami-Ashigara (JP); **Kiyoshi Morimoto**, Minami-Ashigara (JP); **Koichi Yokota**, Minami-Ashigara (JP); **Masahiko Taniguchi**, Minami-Ashigara (JP); **Terukazu Yanagi**, Minami-Ashigara (JP)

(73) Assignee: **Fuji Photo Film Co., Ltd.**, Kanagawa (JP)

(\*) Notice: Subject to any disclaimer, the term of this patent is extended or adjusted under 35 U.S.C. 154(b) by 0 days.

(21) Appl. No.: 10/947,196

(22) Filed: Sep. 23, 2004

(65) **Prior Publication Data**

US 2005/0069824 A1 Mar. 31, 2005

(30) **Foreign Application Priority Data**

Sep. 25, 2003 (JP) 2003-332628

(51) **Int. Cl.**

*G03C 1/815* (2006.01)  
*G03C 1/825* (2006.01)  
*G03C 1/85* (2006.01)  
*G03C 1/46* (2006.01)  
*G03C 3/02* (2006.01)

(52) **U.S. Cl.** 430/512; 430/527; 430/529; 430/631; 430/635; 430/501; 430/507; 430/634

(58) **Field of Classification Search** 430/512, 430/527, 529, 631, 635, 501, 507, 634  
See application file for complete search history.

(56) **References Cited**

U.S. PATENT DOCUMENTS

5,747,235 A 5/1998 Farid et al.

6,689,554 B1 2/2004 Yamada et al.  
6,855,488 B1 \* 2/2005 Yamada et al. .... 430/566  
2004/0018458 A1 \* 1/2004 Nakagawa .... 430/619  
2004/0137386 A1 7/2004 Yokota et al.

\* cited by examiner

Primary Examiner—Geraldine Letscher

(74) Attorney, Agent, or Firm—Sughrue Mion, PLLC

(57) **ABSTRACT**

A silver halide color photosensitive material comprises a blue-sensitive layer, a green-sensitive layer, a red-sensitive layer and a non-light-sensitive layer on a support. The silver halide color photosensitive material contains a compound selected from the following type 1 and type 2 compounds, and wherein the blue-sensitive layer meets the relationship of the following formula (I):

$$S_B(370 \text{ nm})/S_B(420 \text{ nm}) < 0.7 \quad (\text{I})$$

wherein  $S_B(\lambda)$  represents a spectral sensitivity at a wavelength of  $\lambda$ ,

(type 1)

a compound capable of undergoing a one-electron oxidation to thereby form a one-electron oxidation product thereof, wherein the one-electron oxidation product is capable of releasing further one or more electrons accompanying a subsequent bond cleavage reaction, and

(type 2)

a compound capable of undergoing a one-electron oxidation to thereby form a one-electron oxidation product thereof, wherein the one-electron oxidation product is capable of releasing further one or more electrons accompanying a subsequent bond-forming reaction.

**3 Claims, No Drawings**

## SILVER HALIDE COLOR PHOTOSENSITIVE MATERIAL

## CROSS-REFERENCE TO RELATED APPLICATIONS

This application is based upon and claims the benefit of priority from prior Japanese Patent Application No. 2003-332628, filed Sep. 25, 2003, the entire contents of which are incorporated herein by reference.

## BACKGROUND OF THE INVENTION

## 1. Field of the Invention

The present invention relates to a silver halide color photosensitive material of high speed improved with respect to static-induced fog and radiation-induced fog, and relates to a silver halide color photosensitive material which can reduce cissing occurring at high-speed coating, etc. and can be produced stably.

## 2. Description of the Related Art

Various techniques have been employed for enhancing the photo-sensitivity of silver halide photosensitive materials.

Recently, the technique of sensitizing with the use of a compound capable of being one-electron oxidized to thereby form a one-electron oxidation product which by the subsequent bond cleavage reaction, can further emit one electron has been reported (see, for example, Jpn. Pat. Appln. KOKAI Publication No. (hereinafter referred to as JP-A-) 9-211769 and U.S. Pat. No. (hereinafter referred to as "USP") 5,747,235). Moreover, the technique of sensitizing with the use of a compound capable of being one-electron oxidized to thereby form a one-electron oxidation product which by the subsequent bond cleavage reaction, can further emit one electron or more electrons has been reported (see, for example, JP-A's-2003-114487 and 2003-114488).

On the other hand, with respect to photosensitive materials, the greater the enhancement of sensitivity, the more serious the problem of photographic characteristics deterioration by prolonged storage. The causes of the photographic characteristics deterioration by prolonged storage involve not only hitherto well-known heat and moisture but also natural radiation (environmental radiation or cosmic rays). The photosensitive material having been exposed to natural radiation suffers an increase of fog density and, accompanying the same, a deterioration of graininess. The silver halide photosensitive materials having the sensitivity enhanced by the techniques described in the above literature suffer intense radiation-induced fog, so that improvement has been desired thereto.

The photosensitive materials are brought into contact with various materials during the production, use for shooting and development processing thereof. For example, when a photosensitive material is in wound form during the processing, the back layer provided on the back side of the support may be brought into contact with the surface layer. Further, while being conveyed during the processing, the photosensitive material may be brought into contact with stainless steel, rubber rollers, etc. When brought into contact with these materials, the photosensitive material at the surface (gelatin layer) thereof is likely to have positive charge and occasionally induces unwanted electric discharge with the result that undesirable exposure marks (known as static marks) remain on the photosensitive material. Incorporating of a material capable of controlling the spectral sensitivity in the ultraviolet region in the protective layer is

known as means for reducing undesirable exposure marks on the photosensitive material even when unwanted discharge occurs.

The photosensitive materials having been sensitized by the use of compounds as the above spectral sensitivity controlling material pose a problem of static-induced fog.

## BRIEF SUMMARY OF THE INVENTION

10 It is an object of the present invention to provide a silver halide photosensitive material which realizes high sensitivity and which can suppress static-induced fog and radiation-induced fog.

15 While conducting extensive and intensive studies with a view toward obtaining a photosensitive material improved with respect to static-induced fog through appropriate use of an ultraviolet absorber so as to lower the sensitivity in the ultraviolet region in order to effect suppression of static-induced fog, surprisingly, the inventor has found that a 20 photosensitive material improved with respect to not only static-induced fog but also radiation-induced fog can be obtained.

The above object has been attained by the following means.

25 (I) A silver halide color photosensitive material comprising at least one each of a blue-sensitive layer, a green-sensitive layer, a red-sensitive layer and a non-light-sensitive layer on a support, wherein the silver halide color photosensitive material contains a compound selected from 30 among the following type 1 and type 2 compounds, and wherein the blue-sensitive layer meets the relationship of the following formula (I):

$$S_B(370 \text{ nm})/S_B(420 \text{ nm}) < 0.7 \quad (\text{I})$$

35 wherein  $S_B(\lambda)$  represents a spectral sensitivity at a wavelength of  $\lambda$ ,

(Type 1)

40 a compound capable of undergoing a one-electron oxidation to thereby form a one-electron oxidation product thereof, wherein the one-electron oxidation product is capable of releasing further one or more electrons accompanying a subsequent bond cleavage reaction, and

(Type 2)

45 a compound capable of undergoing a one-electron oxidation to thereby form a one-electron oxidation product thereof, wherein the one-electron oxidation product is capable of releasing further one or more electrons accompanying a subsequent bond-forming reaction.

50 (II) The silver halide color photosensitive material according to item (I) above, wherein the silver halide color photosensitive material further contains at least one fluorinated surfactant selected from the group consisting of compounds represented by general formula (A) and compounds represented by general formula (B):

General formula (A)



In the general formula (A), each of  $R^{B3}$ ,  $R^{B4}$  and  $R^{B5}$  independently represents a hydrogen atom or substituent. Each of A and B independently represents a fluorine atom or hydrogen atom. Each of  $n^{B3}$  and  $n^{B4}$  is independently an integer of 4 to 8. Each of  $L^{B1}$  and  $L^{B2}$  independently represents a substituted or unsubstituted alkylene group, substituted or unsubstituted alkyleneoxy group, or bivalent linking group composed of a combination thereof.  $m^B$  is 0 or 1. M represents a cation.



In the general formula (B),  $R^{C1}$  represents a substituted or unsubstituted alkyl group, provided that the substituent does not include a fluorine atom.  $R^{CF}$  represents a perfluoroalkylene group. A represents a hydrogen atom or fluorine atom.  $L^{C1}$  represents a substituted or unsubstituted alkylene group, substituted or unsubstituted alkyleneoxy group, or bivalent linking group composed of a combination thereof. One of  $Y^{C1}$  and  $Y^{C2}$  represents a hydrogen atom while the other represents  $-L^{C2}-SO_3M$  in which  $L^{C2}$  represents a single bond or a substituted or unsubstituted alkylene group and M represents a cation.

Additional objects and advantages of the invention will be set forth in the description which follows, and in part will be obvious from the description, or may be learned by practice of the invention. The objects and advantages of the invention may be realized and obtained by means of the instrumentalities and combinations particularly pointed out hereinafter.

#### DETAILED DESCRIPTION OF THE INVENTION

The compounds of types 1 and 2 contained in the silver halide color photosensitive material of the present invention will be described below.

##### (Type 1)

A compound capable of undergoing a one-electron oxidation to thereby form a one-electron oxidation product thereof, wherein the one-electron oxidation product is capable of releasing further one or more electrons accompanying a subsequent bond cleavage reaction; and

##### (Type 2)

A compound capable of undergoing a one-electron oxidation to thereby form a one-electron oxidation product thereof, wherein the one-electron oxidation product is capable of releasing further one or more electrons accompanying a subsequent bond-forming reaction.

First, the compound of type 1 will be described.

Among the compounds of type 1, examples of the compounds capable of undergoing a one-electron oxidation to thereby form a one-electron oxidation product thereof, wherein the one-electron oxidation product is capable of releasing further one electron accompanying a subsequent bond cleavage reaction are compounds described as "one photon two electrons sensitizers" or "deprotonating electron-donating sensitizers" in the patent publications and

specifications of, for example, JP-A-9-211769 (compounds PMT-1 to S-37 listed in Tables E and F on pages 28 to 32), JP-A-9-211774, JP-A-11-95355 (compounds INV 1 to 36), Japanese Patent Application KOHYO Publication 2001-500996 (compounds 1 to 74, 80 to 87 and 92 to 122), U.S. Pat. Nos. 5,747,235 and 5,747,236, EP 786692A1 (compounds INV 1 to 35), EP 893732A1 and U.S. Pat. Nos. 6,054,260 and 5,994,051, the entire contents of which are incorporated herein by reference. Preferable scopes of these 10 compounds are the same as the preferable scopes described in the referred patent specifications.

Further, as the compound capable of undergoing a one-electron oxidation to thereby form a one-electron oxidation product thereof, wherein the one-electron oxidation product is capable of releasing further one or more electrons accompanying a subsequent bond cleavage reaction includes compounds represented by the general formula (1) (having the same meaning as the general formula (1) described in JP-A-2003-114487), the general formula (2) (having the same meaning as the general formula (2) described in JP-A-2003-114487), the general formula (3) (having the same meaning as the general formula (1) described in JP-A-2003-114488), the general formula (4) (having the same meaning as the general formula (2) described in JP-A-2003-114488), the general formula (5) (having the same meaning as the general formula (3) described in JP-A-2003-114488), the general formula (6) (having the same meaning as the general formula (1) described in JP-A-2003-75950), the general formula (7) (having the same meaning as the general formula (2) described in JP-A-2003-75950), the general formula (8) (having the same meaning as the general formula (1) described in Japanese Patent Application No. 2003-25886), and compounds represented by the general formula (9) (having the same meaning as the general formula (3) described in Japanese Patent Application No. 2003-33446) included among the compounds capable of undergoing the chemical reaction of the formula (1) (having the same meaning as the chemical reaction formula (1) described in Japanese Patent Application No. 2003-33446, 20 the entire contents which disclose the compound of type a mentioned above are incorporated herein by reference. Preferable scopes of these compounds are the same as the preferable scopes described in the referred patent specifications.



In the general formulas (1) and (2),  $RED_1$  and  $RED_2$  each represent a reducing group.  $R_1$  represents a nonmetallic atomic group capable of forming, together with carbon atom (C) and  $RED_1$ , a cyclic structure corresponding to a tetrahydro form, or octahydro form of a 5-membered or 6-membered aromatic ring (including an aromatic heterocycle).  $R_2$ ,  $R_3$ , and  $R_4$  each represents a hydrogen atom or substituent.  $Lv_1$  and  $Lv_2$  each represent a split-off group. ED represents an electron-donating group.



In the general formulas (3), (4) and (5) Z<sub>1</sub> represents an atomic group capable of forming a 6-membered ring together with the nitrogen atom and the two carbon atoms of the benzene ring. R<sub>5</sub>, R<sub>6</sub>, R<sub>7</sub>, R<sub>9</sub>, R<sub>10</sub>, R<sub>11</sub>, R<sub>13</sub>, R<sub>14</sub>, R<sub>15</sub>, R<sub>16</sub>, R<sub>17</sub>, R<sub>18</sub> and R<sub>19</sub> each represent a hydrogen atom or substituent. R<sub>20</sub> represents a hydrogen atom or substituent, provided that when R<sub>20</sub> represents a group other than an aryl group, R<sub>16</sub> and R<sub>17</sub> bond together to form an aromatic ring or aromatic hetero ring. R<sub>8</sub> and R<sub>12</sub> each represent a substituent capable of substituting on the benzene ring. m<sub>1</sub> represents an integer of 0 to 3, and m<sub>2</sub> represents an integer of 0 to 4. LV3, LV4, and LV5 each represent a splitting-off group.



In the general formula (8), RED<sub>5</sub> represents a reducing group, which includes an arylamino group or heterocyclamino group. R<sub>31</sub> represents a hydrogen atom or substituent. X represents an alkoxy group, aryloxy group, heterocyclicoxy group, alkylthio group, arylthio group, heterocyclic thio group, alkylamino group, arylamino group or heterocyclamino group. Lv<sub>6</sub> represents a splitting-off group, which includes a carboxy group or salt thereof, or a hydrogen atom.



General formula (6)



General formula (7)



In the general formulas (6) and (7), RED<sub>3</sub> and RED<sub>4</sub> each represent a reducing group. R<sub>21</sub> to R<sub>30</sub> each represent a hydrogen atom or substituent. Z<sub>2</sub> represents  $-\text{CR}_{111}\text{R}_{112}-$ ,  $-\text{NR}_{113}-$ , or  $-\text{O}-$ . R<sub>111</sub> and R<sub>112</sub> each independently represent a hydrogen atom or substituent. R<sub>113</sub> represents a hydrogen atom, alkyl group, aryl group or heterocyclic group.

45  
The compound represented by the general formula (9) is one that, after undergoing through two-electron oxidation accompanying decarboxylation, undergoes the bond-forming reaction represented by the chemical reaction of 50 (1). In the chemical reaction formula (1), R<sub>32</sub> and R<sub>33</sub> each represents a hydrogen atom or substituent. Z<sub>3</sub> represents a group to form a 5-membered or 6-membered hetero ring together with C=C. Z<sub>4</sub> represents a group to form a 5-membered or 6-membered aryl group or heterocyclic group 55 together with C=C. M represents a radical, radical ion or cation. In the general formula (9), R<sub>32</sub>, R<sub>33</sub>, and Z<sub>3</sub> have the same meaning as those in the chemical reaction formula (1), respectively. Z<sub>5</sub> represents a group to form a 5-membered or 6-membered cyclic aliphatic hydrocarbon group or heterocyclic group together with C=C.

Now the compound of type 2 will be described.

Examples of the compounds of type 2 that is capable of undergoing a one-electron oxidation to thereby form a one-electron oxidation product thereof, wherein the one-electron oxidation product is capable of releasing further one or more electrons accompanying a subsequent bond-forming reaction, are those represented by the general formula (1)

(having the same meaning as the general formula (1) of JP-A-2003-140287), and those capable of undergoing the chemical reaction formula (1) (having the same meaning as the chemical reaction formula (1) of Japanese Patent Application No. 2003-140287) and represented by the general formula (11) (having the same meaning as the general formula (2) of Japanese Patent Application No. 2003-33446). Preferable scopes of these compounds are the same as the preferable scopes described in the referred patent specifications.

RED<sub>6</sub>-Q-Y

General formula (10)

In the general formula (10), RED<sub>6</sub> represents a reducing group capable of undergoing one-electron oxidation. Y represent a reactive group having a carbon-carbon double bond moiety, carbon-carbon triple bond moiety, aromatic moiety or benzo-condensed nonaromatic heterocyclic group, and capable of reacting with a one-electron oxidation product formed as a result of a one-electron oxidation of RED<sub>6</sub> to thereby form a new bond. Q represents a linking group to link RED<sub>6</sub> and Y.



The compound represented by the general formula (11) is one that undergoes, by being oxidized, the bond-forming reaction represented by the chemical reaction formula (1). In the chemical reaction formula (1), R<sub>32</sub> and R<sub>33</sub> each represent a hydrogen atom or substituent. Z<sub>3</sub> represents a group to for a 5-membered or 6-membered hetero ring together with C=C. Z<sub>4</sub> represents a group to for a 5-membered or 6-membered aryl group or heterocyclic group together with C=C. Z<sub>5</sub> represents a group to form a 5-membered or 6-membered cyclic aliphatic hydrocarbon group or heterocyclic group. M represents a radical, radical ion or cation. In the general formula (11), R<sub>32</sub>, R<sub>33</sub>, Z<sub>3</sub> and Z<sub>4</sub> have the same meaning as those in the chemical reaction formula (1), respectively.

Among the compounds of types 1 and 2, "a compound having an adsorptive group to silver halide in a molecular" or "a compound having a partial structure of a spectrally sensitizing dye in a molecular" is preferable. Representative ones of the adsorptive group to silver halide are the groups

described in the specification on page 16, right column, line 1 to page 17, right column line 12 of JP-A-2003-156823. The partial structure of the spectrally sensitizing dye is the structure described on page 17, right column, line 34 to page 18, left column, line 6 of the same specification, the entire contents of which are incorporated herein by reference.

As the compounds of types 1 and 2 "a compound having at least one adsorptive group to silver halide in a molecular" is preferable. "A compound having at least two adsorptive groups to silver halide in a molecular" is more preferable. When there are two or more adsorptive groups in a single molecular these adsorptive groups may be the same or different to each other.

As the adsorptive groups preferred ones are nitrogen-containing heterocyclic groups substituted with mercapto (e.g., a 2-mercaptopthiadiazole group, 3-mercaptop-1,2,4-triazole group, 5-mercaptotetrazole group, 2-mercaptop-1,3,4-oxadiazole group, 2-mercaptobenzoxazole group, 2-mercaptobenzothiazole group or 1,5-dimethyl-1,2,4-triazolium-3-thiolate group), or a nitrogen-containing heterocyclic group having an —NH— group capable of forming an iminosilver (>N<sup>+</sup>Ag) as a partial structure of the heterocycle (e.g., a benzotriazole group, benzimidazole group or indazole group). More preferably, the adsorptive group is a 5-mercaptotetrazole group, 3-mercaptop-1,2,4-triazole group or benzotriazole group. Most preferably, the adsorptive group is a 3-mercaptop-1,2,4-triazole group or 5-mercaptotetrazole group.

Among the compounds of the present invention, those having, in its molecule, two or more mercapto groups as partial structures are also especially preferred. Herein, the mercapto group (—SH) may become a thione group when it can be tautomerized. Preferable examples of such compounds possessing in its molecule two or more adsorptive groups as a partial structure (e.g., dimercapto substituted nitrogen-containing heterocyclic group) are 2,4-dimercaptopyrimidine group, 2,4-dimercaptotriazine group, and 3,5-dimercapto-1,2,4-triazole group.

A quaternary salt structure of nitrogen or phosphor may be preferably used as the adsorptive group. The quaternary salt structure of nitrogen specifically is an ammonio group (e.g., trialkylammonio group, dialkylaryl (or heteroaryl) ammonio group, alkyldiaryl (or heteroaryl) ammonio group) or a group containing a nitrogen-containing group including a quaternary nitrogen atom. The quaternary salt structure of phosphor specifically is a phosphonio group (e.g., trialkylphosphonio, dialkylaryl (or heteroaryl) phosphonio, alkyl-diaryl (or heteroaryl) phosphonio group, or triaryl (or heteroaryl) phosphonio). A quaternary salt structure of nitrogen is more preferably used as the adsorptive group, a 5-membered or 6-membered nitrogen-containing aromatic heterocyclic group including a quaternary nitrogen atom is much more preferably used. A pyridinio, quinolinio or isoquinolinio is especially preferably used. These nitrogen-containing heterocyclic group including a quaternary nitrogen atom may have a substituent.

As an example of a counter anion of the quaternary salt, halide ion, carboxylate ion, sulfonate ion, sulfate ion, perchlorate ion, carbonate ion, nitrate ion, BF<sub>4</sub><sup>-</sup>, PF<sub>6</sub><sup>-</sup> or Ph<sub>4</sub>B may be mentioned. When a group having a negative charge is present in carboxylate an etc., in a molecular, a intra molecular salt may be formed together with it. As a counter anion that is not present in a molecular, chloride ion, bromide ion, or methansulfonate ion is especially preferable.

**9**

Preferable examples of the compound represented by types 1 and 2 having a quaternary salt structure of phosphor or nitrogen as an adsorptive group are represented by general formula (X)



General formula (X)

In general formula (X), P and R each independently represent a quaternary salt structure of nitrogen or phosphor that is not a partial structure of a sensitizing dye.  $Q_1$  and  $Q_2$  each independently represent a linking group, specifically a simple bond, alkylene, arylene, heterocyclic group,  $—O—$ ,  $—S—$ ,  $—NR_N—$ ,  $—C(=O)—$ ,  $—SO_2—$ ,  $—SO—$  or  $—P(=O)—$  alone or combination of these groups. Herein,  $R_N$  represents a hydrogen atom, alkyl group, aryl group or

5

**10**

heterocyclic group. S represents a residue of the compound represented by type one or two from which an atom is removed. Each of i and j is an integer of 1 or more, and selected from the scope in which  $i+j$  is 2 to 6. Preferably, i is 1 to 3, and j is 1 to 2. More preferably, i is one or two and j is 1. Especially preferably, i is 1 and j is 1. The compounds represented by the general formula (X) are those having the total carbon atoms within the scope of preferably 10 to 100, more preferably 10 to 70, much more preferably 11 to 60 and especially preferably 12 to 50.

Specific examples of the compounds of types 1 and 2 are set forth below, but the present invention is not limited to these.

1



2



3



4



5



6



**11****12**

-continued

7

8



9



10



11



12

13



14



-continued

15

16



17



18



19



20



21



21



22



-continued



26



27



28



-continued

30

31



32

33



35

35



36

37



38

39



-continued

40

41



42

43



44



45



46



-continued



The compound of type 1 and type 2 may be used at any time during emulsion preparation or in photosensitive material manufacturing step, for example, during grain formation, at desalting step, at the time of chemical sensitization, or before coating. The compound may be added separately in a plurality of times during the steps. Preferable addition timing is from the completion of grain formation to before a desalting step, at the time of chemical sensitization (immediately before the initiation of chemical sensitization to immediately after the completion thereof), or before coating. More preferable addition timing is at chemical sensitization or before coating.

The compound of type 1 and type 2 may preferable be added by dissolving it to a water or water-soluble solvent such as methanol, ethanol or a mixture of solvents. When the compound is added to water, if the solubility of the compound increases in a case where pH is raised or lowered, the compound may be added to the solvent by raising or lowering the pH thereof.

It is preferable that the compound of type 1 and types 2 is used in an emulsion layer, but the compound may be added in a protective layer or interlayer together with the emulsion layer, thereby making the compound diffuse during coating. The addition time of the compound of the invention is irrespective of before or after the addition time of a sensitizing dye. Each of the compounds is preferably contained in a silver halide emulsion layer in an amount of  $1 \times 10^{-9}$  to  $5 \times 10^{-2}$  mol, more preferably  $1 \times 10^{-8}$  to  $2 \times 10^{-3}$  mol pre mol of silver halide.

In the present invention, the terminology "spectral sensitivity distribution" refers to a function of photographic speed versus wavelength, the photographic speed at each wavelength referring to the inverse number of exposure amount capable of realizing a given density at each wavelength when spectral exposure with intervals of several nanometers (nm) from 350 to 700 nm is applied to a silver halide color photosensitive material. In the present invention, the spectral sensitivity distribution of blue-sensitive layer  $S_B(\lambda)$  refers to a sensitivity distribution which realizes yellow density.

In the spectral sensitivity distribution preferred in the present invention, with the spectral sensitivity referring to the inverse number of exposure amount capable of realizing a given density, the spectral sensitivity of blue-sensitive layer  $S_B(\lambda)$  is expressed by the following relationship at wavelengths of 370 nm and 420 nm.

With respect to the following general formulas, although it is satisfactory for the spectral sensitivity at any density to fall within the ranges, it is preferred that the spectral sensitivity at any of the density range from  $D_{min}+0.3$  to  $D_{min}+1.0$  fall within the following ranges. With respect to

the development processing conditions for realizing the spectral sensitivity distribution, although any of common color negative development processing techniques is satisfactory, it is preferred to employ the development processing described in Example 1 of this application.

20  $S_B(370 \text{ nm})/S_B(420 \text{ nm}) < 0.7$ ,

25 preferably

$S_B(370 \text{ nm})/S_B(420 \text{ nm}) < 0.6$ ,

more preferably

30  $S_B(370 \text{ nm})/S_B(420 \text{ nm}) < 0.5$ ,

and most preferably,

35  $S_B(370 \text{ nm})/S_B(420 \text{ nm}) < 0.3$ .

40 A silver halide photosensitive material of unprecedented antistatic performance and excellent high-speed coatability can be provided by incorporation of the fluorinated surfactant represented by the general formula (A) and/or general formula (B) according to the present invention in the coating film.

45 The general formula (A) will be described in detail below.

First, the compound represented by the following general formula (A) will be described in detail.

General formula (A)



50 In the general formula (A), each of  $R^{B3}$ ,  $R^{B4}$  and  $R^{B5}$  independently represents a hydrogen atom or substituent. Each of A and B independently represents a fluorine atom or hydrogen atom. Each of  $n^{B3}$  and  $n^{B4}$  is independently an integer of 4 to 8. Each of  $L^{B1}$  and  $L^{B2}$  independently represents a substituted or unsubstituted alkylene group, substituted or unsubstituted alkyleneoxy group, or bivalent linking group composed of a substituted or unsubstituted alkylene group combined with a substituted or unsubstituted alkyleneoxy group.  $m^B$  is 0 or 1. M represents a cation.

23

In the general formula (A), each of  $R^{B3}$ ,  $R^{B4}$  and  $R^{B5}$  independently represents a hydrogen atom or substituent. Any of the substituents described as T to be referred to later can be used as the substituent.

Each of  $R^{B3}$ ,  $R^{B4}$  and  $R^{B5}$  preferably represents an alkyl group or hydrogen atom; more preferably an alkyl group having 1 to 12 carbon atoms or hydrogen atom; still more preferably a methyl group or hydrogen atom; and most preferably a hydrogen atom.

In the general formula (A), each of A and B independently represents a fluorine atom or hydrogen atom. Preferably, A and B simultaneously represent a fluorine atom or hydrogen atom. More preferably, A and B simultaneously represent a fluorine atom.

In the general formula (A), each of  $n^{B3}$  and  $n^{B4}$  is independently an integer of 4 to 8. Preferably, each of  $n^{B3}$  and  $n^{B4}$  is an integer of 4 to 6, and  $n^{B3}=n^{B4}$ . More preferably, each of  $n^{B3}$  and  $n^{B4}$  is an integer of 4 or 6, and  $n^{B3}=n^{B4}$ . Still more preferably,  $n^{B3}=n^{B4}=4$ .

In the general formula (A),  $m^B$  is 0 or 1, both equally preferred.

In the general formula (A), each of  $L^{B1}$  and  $L^{B2}$  independently represents a substituted or unsubstituted alkylene group, substituted or unsubstituted alkyleneoxy group, or bivalent linking group composed of a substituted or unsubstituted alkylene group combined with a substituted or unsubstituted alkyleneoxy group. Any of the substituents described as T to be referred to later can be used as the substituent.

Each of  $L^{B1}$  and  $L^{B2}$  is preferably a group having 4 or less carbon atoms, and is preferably an unsubstituted alkylene.

M represents a cation. As the cation represented by M, preferred use is made of, for example, an alkali metal ion (lithium ion, sodium ion, potassium ion, etc.), an alkaline earth metal ion (barium ion, calcium ion, etc.), or ammonium ion. Lithium ion, sodium ion, potassium ion and ammonium ion are preferred. Lithium ion, sodium ion and potassium ion are more preferred. Sodium ion is still more preferred.

Among the compounds of the above general formula (A), compounds of the following general formula (A-1) are preferred.

General formula (A-1)



In the general formula (A-1),  $R^{B3}$ ,  $R^{B4}$ ,  $R^{B5}$ ,  $n^{B3}$ ,  $n^{B4}$ ,  $m^B$ , A, B and M are as defined above with respect to the general formula (A). Preferred ranges thereof are also the same as mentioned above. Each of  $n^{B1}$  and  $n^{B2}$  is independently an integer of 1 to 6.

In the general formula (A-1), each of  $n^{B1}$  and  $n^{B2}$  is independently an integer of 1 to 6. Preferably, each of  $n^{B1}$  and  $n^{B2}$  is an integer of 1 to 6, and  $n^{B1}=n^{B2}$ . More preferably, each of  $n^{B1}$  and  $n^{B2}$  is an integer of 2 or 3, and  $n^{B1}=n^{B2}$ . Still more preferably,  $n^{B1}=n^{B2}=2$ .

24

Among the compounds of the above general formula (A), compounds of the following general formula (A-2) are more preferred.

5

General formula (A-2)



10

20

15

In the general formula (A-2),  $n^{B3}$ ,  $n^{B4}$ ,  $m^B$  and M are as defined above with respect to the general formula (A). Preferred ranges thereof are also the same as mentioned above. In the general formula (A-2),  $n^{B1}$  and  $n^{B2}$  are as defined above with respect to the general formula (A-1). Preferred ranges thereof are also the same as mentioned above.

25

Among the compounds of the above general formula (A), compounds of the following general formula (A-3) are still more preferred.

30

General formula (A-3)



40

45

In the general formula (A-3),  $n^{B5}$  is 2 or 3, and  $n^{B6}$  is an integer of 4 to 6.  $m^B$  is 0 or 1, both equally preferred. M is as defined above with respect to the general formula (A). Preferred range thereof is also the same as mentioned above.

Specific examples of the compounds of the above general formula (A) will be shown below, which however in no way limit the scope of the present invention.

50

FS-201



55

FS-202



-continued



-continued





-continued



-continued

FS-241



FS-242



FS-243



FS-244



The compounds of the above general formula (A) can be easily synthesized by the use of common esterification reaction and sulfonation reaction in combination. The conversion of counter cation can be easily accomplished by the use of an ion exchange resin. Examples of representative synthetic methods will be described below, which however in no way limit the scope of the present invention.

## SYNTHETIC EXAMPLE 1

## Synthesis of Compound FS-201

FS-239 50 1-1 Synthesis of di(3,3,4,4,5,5,6,6,6-nonafluorohexyl)maleate

90.5 g (0.924 mol) of maleic anhydride, 500 g (1.89 mol) of 3,3,4,4,5,5,6,6-nonafluorohexanol and 17.5 g (0.09 mol) of p-toluenesulfonic acid monohydrate were heated in 1000 L of toluene under reflux while distilling off formed water for 20 hr. The thus obtained reaction mixture was cooled to room temperature, and toluene was added thereto. The organic phase was washed with water, and the solvent was distilled off in vacuum, thereby obtaining 484 g of desired product (yield 86%) as a transparent liquid.

FS-240 60 1-2 Synthesis of Compound FS-201

514 g (0.845 mol) of di(3,3,4,4,5,5,6,6,6-nonafluorohexyl)maleate, 91.0 g (0.875 mol) of sodium hydrogen sulfite and 250 mL of water/ethanol (1/1 v/v) were mixed together, and heated under reflux for 6 hr. 500 mL of ethyl acetate and 120 mL of a saturated aqueous solution of sodium chloride were added to the mixture, and an extrac-

tion was effected. The organic phase was recovered, and sodium sulfate was added so as to dehydrate the organic phase. Sodium sulfate was removed by filtration, and the filtrate was concentrated. 2.5 L of acetone was added to the concentrate, and heated. Undissolved matter was filtered off, and the solution was cooled to 0° C. 2.5 L of acetonitrile was slowly added to effect precipitation. Precipitated solid was collected by filtration, and obtained crystal was dried in vacuum at 80° C. As a result, 478 g (yield 79%) of desired compound as white crystal was obtained. <sup>1</sup>H-NMR data of the obtained compound are as follows:

<sup>1</sup>H-NMR (DMSO-d<sub>6</sub>) δ 2.49–2.62 (m, 4H), 2.85–2.99 (m, 2H), 3.68 (dd, 1H), 4.23–4.35 (m, 4H).

Now, the compounds of the following general formula (B) will be described in detail.

General formula (B)



In the general formula (B), R<sup>C1</sup> represents a substituted or unsubstituted alkyl group (provided that the substituent does not include a fluorine atom). R<sup>CF</sup> represents a perfluoroalkylene group. A represents a hydrogen atom or fluorine atom. L<sup>C1</sup> represents a substituted or unsubstituted alkylene group, a substituted or unsubstituted alkyleneoxy group, or bivalent linking group composed of a combination of a substituted or unsubstituted alkylene group with a substituted or unsubstituted alkyleneoxy group. One of Y<sup>C1</sup> and Y<sup>C2</sup> represents a hydrogen atom while the other represents -L<sup>C2</sup>-SO<sub>3</sub>M in which L<sup>C2</sup> represents a single bond or a substituted or unsubstituted alkylene group and M represents a cation.

In the general formula (B), R<sup>C1</sup> represents a substituted or unsubstituted alkyl group. The substituted or unsubstituted alkyl group represented by R<sup>C1</sup> may be linear, or may be in the form of a branched chain, or may have a cyclic structure. Any of the substituents described as T to be referred to later can be used as the substituent. As the substituent, there can preferably be mentioned an alkenyl group, aryl group, alkoxy group, halogen atom (more preferably Cl), carboxylic ester group, carbonamido group, carbamoyl group, oxy-carbonyl group, phosphoric ester group or the like.

R<sup>C1</sup> preferably represents an unsubstituted alkyl group, more preferably an unsubstituted alkyl group having 2 to 24 carbon atoms, still more preferably an unsubstituted alkyl group having 4 to 20 carbon atoms, and especially preferably an unsubstituted alkyl group having 6 to 20 carbon atoms.

R<sup>CF</sup> represents a perfluoroalkylene group. Herein, the perfluoroalkylene group refers to an alkylene group having all the hydrogen atoms thereof replaced by fluorine. The perfluoroalkylene group may be linear, or may be in the form of a branched chain, or may have a cyclic structure. R<sup>CF</sup> preferably has 1 to 10 carbon atoms, more preferably 1 to 8 carbon atoms.

A represents a hydrogen atom or fluorine atom. A fluorine atom is preferred.

L<sup>C1</sup> represents a substituted or unsubstituted alkylene group, substituted or unsubstituted alkyleneoxy group, or a

bivalent group composed of a combination of a substituted or unsubstituted alkylene group with a substituted or unsubstituted alkyleneoxy group. The substituent can be any of those of preferred range which have been mentioned above with respect to R<sup>C1</sup>. L<sup>C1</sup> preferably has 4 or less carbon atoms, and it is preferred that L<sup>C1</sup> represent an unsubstituted alkylene.

One of Y<sup>C1</sup> and Y<sup>C2</sup> represents a hydrogen atom while the other represents -L<sup>C2</sup>-SO<sub>3</sub>M in which M represents a cation.

10 As the cation represented by M, preferred use is made of, for example, an alkali metal ion (lithium ion, sodium ion, potassium ion, etc.), an alkaline earth metal ion (barium ion, calcium ion, etc.), or ammonium ion. Lithium ion, sodium ion, potassium ion and ammonium ion are more preferred.

15 Lithium ion, sodium ion and potassium ion are still more preferred. Appropriate cation can be selected depending on the total number of carbon atoms, substituent, degree of alkyl branching, etc. with respect to the compound of the above general formula (B). When the total number of carbon

20 atoms had by R<sup>C1</sup>, R<sup>CF</sup> and L<sup>C1</sup> is 16 or greater, the employment of lithium ion is advantageous from the viewpoint of simultaneous attainment of solubility (especially in water) and antistatic capability or coating uniformity.

25 L<sup>C2</sup> represents a single bond or a substituted or unsubstituted alkylene group. The substituent can be any of those of preferred range which have been mentioned above with respect to R<sup>C1</sup>.

30 L<sup>C2</sup> preferably represents a single bond or an alkylene group having 2 or less carbon atoms, more preferably a single bond or an unsubstituted alkylene group, and still more preferably a single bond or a methylene group. Most preferably, L<sup>C2</sup> represents a single bond.

35 Among the compounds of the above general formula (B), compounds of the following general formula (B-1) are preferred.

General formula (B-1)



40 In the general formula (B-1), R<sup>C11</sup> represents a substituted or unsubstituted alkyl group whose total number of carbon atoms is 6 or greater. R<sup>CF1</sup> represents a perfluoroalkyl group having 6 or less carbon atoms. One of Y<sup>C11</sup> and Y<sup>C12</sup> represents a hydrogen atom while the other represents SO<sub>3</sub>MC in which MC represents a cation. n<sup>C1</sup> is an integer of 1 or greater.

45 55 In the general formula (B-1), R<sup>C11</sup> represents a substituted or unsubstituted alkyl group whose total number of carbon atoms is 6 or greater, provided that R<sup>C11</sup> is not a fluorinated alkyl group. The substituted or unsubstituted alkyl group represented by R<sup>C11</sup> may be linear, or may be in the form of a branched chain, or may have a cyclic structure. As the substituent, there can be mentioned an alkenyl group, an aryl group, an alkoxy group, a halogen atom excluding fluorine, a carboxylic ester group, a carbonamido group, a carbamoyl group, an oxycarbonyl group, a phosphoric ester group or the like.

60 65 The total number of carbon atoms of the substituted or unsubstituted alkyl group represented by R<sup>C11</sup> is preferably

in the range of 6 to 24. Preferred examples of the unsubstituted alkyl groups having 6 to 24 carbon atoms include n-hexyl, n-heptyl, n-octyl, tert-octyl, 2-ethylhexyl, n-nonyl, 1,1,3-trimethylhexyl, n-decyl, n-dodecyl, cetyl, hexadecyl, 2-hexyldecyl, octadecyl, eicosyl, 2-octyldodecyl, docosyl, tetracosyl, 2-decyldodecyl, tricosyl, cyclohexyl, cycloheptyl and the like. Preferred examples of the substituted alkyl groups whose total number of carbon atoms, inclusive of the carbon atoms of substituent, is in the range of 6 to 24 include 5 10 15 2-hexenyl, oleyl, linoleyl, linolenyl, benzyl,  $\beta$ -phenethyl, 2-methoxyethyl, 4-phenylbutyl, 4-acetoxyethyl, 6-phenoxyhexyl, 12-phenyldodecyl, 18-phenyloctadecyl, 12-(p-chlorophenyl)dodecyl, 2-(phosphatodiphenyl)ethyl and the like.

The total number of carbon atoms of the substituted or 15 unsubstituted alkyl group represented by  $R^{C11}$  is more preferably in the range of 6 to 18. Preferred examples of the unsubstituted alkyl groups having 6 to 18 carbon atoms include n-hexyl, cyclohexyl, n-heptyl, n-octyl, 2-ethylhexyl, n-nonyl, 1,1,3-trimethylhexyl, n-decyl, n-dodecyl, cetyl, 20 hexadecyl, 2-hexyldecyl, octadecyl, 4-tert-butylcyclohexyl and the like. Preferred examples of the substituted alkyl groups whose total number of carbon atoms, inclusive of the carbon atoms of substituent, is in the range of 6 to 18 include phenethyl, 6-phenoxyhexyl, 12-phenyldodecyl, oleyl, linoleyl, linolenyl and the like. Still more preferably,  $R^{C11}$  25 represents n-hexyl, cyclohexyl, n-heptyl, n-octyl, 2-ethylhexyl, n-nonyl, 1,1,3-trimethylhexyl, n-decyl, n-dodecyl, cetyl, hexadecyl, 2-hexyldecyl, octadecyl, oleyl, linoleyl or linolenyl. It is most preferred that  $R^{C11}$  represent a linear, 30 35 40 45 50 carbon atoms.

In the general formula (B-1),  $R^{CF1}$  represents a perfluoroalkyl group having 6 or less carbon atoms. Herein, the perfluoroalkyl group refers to an alkyl group having all the hydrogen atoms thereof replaced by fluorine. The alkyl of the perfluoroalkyl group may be linear, or may be in the form of a branched chain, or may have a cyclic structure. The perfluoroalkyl group represented by  $R^{CF1}$  can be, for example, any of trifluoromethyl, pentafluoroethyl, heptafluoro-n-propyl, heptafluoroisopropyl, nonafluoro-n-butyl, undecafluoro-n-pentyl, tridecafluoro-n-hexyl, undecafluorocyclohexyl and the like. Of these, perfluoroalkyl groups having 2 to 4 carbon atoms (e.g., pentafluoroethyl, heptafluoro-n-propyl, heptafluoroisopropyl and nonafluoro-n-butyl) are preferred. Heptafluoro-n-propyl and nonafluoro-n-butyl are especially preferred.

In the general formula (B-1),  $n^{C1}$  is an integer of 1 or greater, preferably an integer of 1 to 4, and most preferably 1 or 2.

With respect to combinations of  $n^{C1}$  and  $R^{CF1}$ , it is preferred that when  $n^{C1}=1$ ,  $R^{CF1}$  be heptafluoro-n-propyl or nonafluoro-n-butyl, and that when  $n^{C1}=2$ ,  $R^{CF1}$  be non-55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 9900 9905 9910 9915 9920 9925 9930 9935 9940 9945 9950 9955 9960 9965 9970 9975 9980 9985 9990 9995 10000 10005 10010 10015 10020 10025 10030 10035 10040 10045 10050 10055 10060 10065 10070 10075 10080 10085 10090 10095 10100 10105 10110 10115 10120 10125 10130 10135 10140 10145 10150 10155 10160 10165 10170 10175 10180 10185 10190 10195 10200 10205 10210 10215 10220 10225 10230 10235 10240 10245 10250 10255 10260 1

-continued



-continued



30 The compounds of the above general formula (B) can be easily synthesized by sequentially subjecting common maleic anhydride, etc. as a raw material to monoesterification reaction, acid halogenation, esterification reaction and sulfonation reaction. Further, the replacement of counter 35 cation can be easily effected by the use of an ion exchange resin.

Examples of representative synthetic methods will be described below, which however in no way limit the scope of the present invention.

## SYNTHETIC EXAMPLE 2

## Synthesis of Compound FS-303

FS-328 45 2-1 Synthesis of 2-ethylhexyl maleate chloride  
4.5 g (20 mmol) of mono(2-ethylhexyl)maleic

FS-329 50 1.0 g (20 mmol) of maleic(2-ethylhexyl)maleate, product of Aldrich, was slowly dropped in 4.1 g (20 mmol) of phosphorus pentachloride while maintaining the temperature of the mixture at 30° C. or below. After the completion of dropping, the mixture was agitated at room temperature for 1 hr. Thereafter, the mixture was heated to 60° C., and the pressure was reduced by an aspirator to thereby distill off formed phosphorus oxychloride. As a result, there was obtained 4.5 g (yield: 92%) of light brown oily compound consisting of 2-ethylhexyl maleate chloride.

FS-330 55

2-2 Synthesis of mono(2-ethylhexyl)mono(2,2,3,3,4,4,4-heptafluorobutyl)maleate

66.8 g (0.334 mol) of 2,2,3,3,4,4,4-heptafluorobutanol and 29.6 mL (0.367 mol) of pyridine were dissolved in 180 mL of acetonitrile, and while maintaining the internal temperature at 20° C. or below by cooling with an ice bath, 90.6 g (0.367 mol) of mono(2-ethylhexyl)maleate chloride was dropped in the solution. After the completion of dropping, the mixture was agitated at room temperature for 1 hr. Thereafter, 1000 mL of ethyl acetate was added, and the organic phase was washed with a 1 mol/L aqueous hydro-

chloric acid solution and a saturated aqueous sodium chloride solution. The resultant organic layer was collected, and the organic solvent was distilled off in vacuum. Purification by silica gel column chromatography (hexane/chloroform: 10/0 to 7/3 v/v) was performed, thereby obtaining 80.3 g (yield: 59%) of desired compound as a colorless transparent oily compound.

2-3 Synthesis of sodium mono(2-ethylhexyl)mono(2,2,3,3,4,4,4-heptafluorobutyl)sulfosuccinate (FS-303)

80.3 g (0.196 mol) of mono(2-ethylhexyl)mono(2,2,3,3,4,4,4-heptafluorobutyl)maleate, 20.4 g (0.196 mol) of sodium hydrogen sulfite and 80 mL of water/ethanol (1/1 v/v) were mixed together and heated under reflux for 10 hr. Thereafter, 1000 mL of ethyl acetate was added, and the organic phase was washed with a saturated aqueous sodium chloride solution. The resultant organic layer was collected, and the organic solvent was distilled off in vacuum. Purification by silica gel column chromatography (chloroform/methanol: 9/1 v/v) was performed. The collected organic phase was washed with a saturated aqueous sodium chloride solution, and the organic solvent was distilled off in vacuum, thereby obtaining 32 g (yield: 32%) of desired compound as a colorless transparent solid.

<sup>1</sup>H-NMR data of the obtained compound are as follows:

<sup>1</sup>H-NMR (DMSO-d<sub>6</sub>) δ 0.81–0.87 (m, 6H), 1.24 (m, 8H), 1.50 (b r, 1H), 2.77–2.99 (m, 2H), 3.63–3.71 (m, 1H), 3.86–3.98 (m, 3H), 4.62–4.84 (br, 1H).

SYNTHETIC EXAMPLE 3

Synthesis of Compound FS-312

3-1 Synthesis of monodecyl mono(3,3,4,4,5,5,6,6,6-nonafluorohexyl)maleate

164.6 g (623 mmol) of 3,3,4,4,5,5,6,6,6-nonafluorohexanol and 49.3 mL (623 mmol) of pyridine were dissolved in 280 mL of chloroform, and while maintaining the internal temperature at 20° C. or below by cooling with an ice bath, 155.8 g (566 mmol) of monodecyl maleate chloride was dropped in the solution. After the completion of dropping, the mixture was agitated at room temperature for 1 hr. Thereafter, ethyl acetate was added, and the organic phase was washed with a 1 mol/L aqueous hydrochloric acid solution and a saturated aqueous sodium chloride solution. The resultant organic layer was collected, and the organic solvent was distilled off in vacuum. Purification by silica gel column chromatography (hexane/chloroform: 10/0 to 7/3 v/v) was performed, thereby obtaining 48.2 g (yield: 18%) of desired compound.

3-2 Synthesis of sodium monodecyl mono(3,3,4,4,5,5,6,6-nonafluorohexyl)sulfosuccinate (FS-312)

48.0 g (90 mmol) of monodecyl mono(3,3,4,4,5,5,6,6-nonafluorohexyl)maleate, 10.4 g (99 mmol) of sodium hydrogen sulfite and 50 mL of water/ethanol (1/1 v/v) were mixed together and heated under reflux for 5 hr. Thereafter, ethyl acetate was added, and the organic phase was washed with a saturated aqueous sodium chloride solution. The resultant organic layer was collected, and the organic solvent was distilled off in vacuum. Recrystallization from acetonitrile was performed, thereby obtaining 12.5 g (yield: 22%) of desired compound as a colorless transparent solid.

<sup>1</sup>H-NMR data of the obtained compound are as follows:

<sup>1</sup>H-NMR (DMSO-d<sub>6</sub>) δ 0.81–0.87 (t, 3H), 1.24 (m, 18H), 1.51 (br, 2H), 2.50–2.70 (m, 2H), 2.70–2.95 (m, 2H), 3.61–3.70 (m, 1H), 3.96 (m, 2H), 4.28 (ms, 2H).

SYNTHETIC EXAMPLE 4

Synthesis of Compound FS-309

5 4-1 Synthesis of mono(2-ethylhexyl)mono(3,3,4,4,5,5,6,6,6-nonafluorohexyl)maleate

515 g (1.95 mol) of 3,3,4,4,5,5,6,6,6-nonafluorohexanol, 169 g (2.13 mol) of pyridine and 394 mL (3.89 mol) of triethylamine were dissolved in 1000 mL of chloroform, and while maintaining the internal temperature at 20° C. or below by cooling with an ice bath, 530 g (2.14 mol) of 2-ethylhexyl maleate chloride was dropped in the solution. After the completion of dropping, the mixture was agitated at room temperature for 1 hr. Thereafter, chloroform was added, and the organic phase was washed with water and a saturated aqueous sodium chloride solution. The resultant organic layer was collected, and the organic solvent was distilled off in vacuum. Purification by silica gel column chromatography (hexane/chloroform: 10/0 to 7/3 v/v) was performed, thereby obtaining 508 g (yield: 50%) of colorless transparent desired compound.

4-2 Synthesis of sodium mono(2-ethylhexyl)mono(3,3,4,4,5,5,6,6,6-nonafluorohexyl)sulfosuccinate (FS-309)

25 137.5 g (0.29 mol) of mono(2-ethylhexyl)mono(3,3,4,4,5,5,6,6,6-nonafluorohexyl)maleate, 33.2 g (0.32 mol) of sodium hydrogen sulfite and 140 mL of water/ethanol (1/1 v/v) were mixed together and heated under reflux for 2 hr. Thereafter, 1000 mL of ethyl acetate was added, and the organic phase was washed with a saturated aqueous sodium chloride solution. The resultant organic layer was collected, and the organic solvent was distilled off in vacuum. Recrystallization from 800 mL of toluene was performed. Crystal was precipitated by cooling with an ice bath, and finally collected by filtration. As a result, there was obtained 140 g (yield: 84%) of colorless transparent desired compound.

<sup>1</sup>H-NMR data of the obtained compound are as follows:

<sup>1</sup>H-NMR (DMSO-d<sub>6</sub>) δ 0.82–0.93 (m, 6H), 1.13–1.32 (m, 8H), 1.50 (br, 1H), 2.57–2.65 (m, 2H), 2.84–2.98 (m, 2H), 3.63–3.68 (m, 1H), 3.90 (d, 2H), 4.30 (m, 2H).

SYNTHETIC EXAMPLE 5

Synthesis of Compound FS-332

45 5-1 Synthesis of mono(2-ethylhexyl)mono(1,1,1,3,3,3-hexafluoro-2-propyl)maleate

50 33.7 g (201 mmol) of 1,1,1,3,3,3-hexafluoro-2-propanol (HFIP) and 17.9 mL (220 mmol) of pyridine were dissolved in 80 mL of acetonitrile, and while maintaining the internal temperature at 20° C. or below by cooling with an ice bath, 41.8 g (220 mmol) of mono(2-ethylhexyl)maleate chloride was dropped in the solution. After the completion of dropping, the mixture was agitated at room temperature for 1 hr. Thereafter, ethyl acetate was added, and the organic phase was washed with a 1 mol/L aqueous hydrochloric acid solution and a saturated aqueous sodium chloride solution. The resultant organic layer was collected, and the organic solvent was distilled off in vacuum. Purification by silica gel column chromatography (hexane/chloroform: 10/0 to 7/3 v/v) was performed, thereby obtaining 10.6 g (yield: 14%) of desired compound as a colorless transparent oily compound.

65 5-2 Synthesis of Compound FS-332

10.6 g (28 mmol) of mono(2-ethylhexyl)mono(1,1,1,3,3,3-hexafluoro-2-propyl)maleate, 3.2 g (31 mmol) of sodium

hydrogen sulfite and 10 mL of water/ethanol (1/1 v/v) were mixed together and heated under reflux for 10 hr. Thereafter, ethyl acetate was added, and the organic phase was washed with a saturated aqueous sodium chloride solution. The resultant organic layer was collected, and the organic solvent was distilled off in vacuum. Recrystallization from acetonitrile was performed, thereby obtaining 1.7 g (yield: 13%) of desired compound as a colorless transparent solid.

<sup>1</sup>H-NMR data of the obtained compound are as follows:

<sup>1</sup>H-NMR (DMSO-d<sub>6</sub>) δ 0.81–0.87 (m, 6H), 1.25 (m, 8H), 1.50 (br, 1H), 2.73–2.85 (m, 2H), 3.59 (m, 1H), 3.85–3.90 (m, 2H), 12.23 (br, 1H).

Among the above various compounds, ionic surfactants can be used in the form of various salts produced by ion exchange, neutralization or other means, or used in the presence of at least one counter ion, in accordance with the purpose of use thereof, needed properties, etc.

The layer to be loaded with the fluorinated compound of the present invention and the amount thereof are not particularly limited. The use amount thereof can be arbitrarily decided in conformity with the structure and usage of employed compound, the type and amount of materials contained in water-base composition, the constitution of medium, etc. For example, when it is intended to use the water-base coating composition of the present invention as a coating liquid for the hydrophilic colloid (gelatin) layer constituting the uppermost layer of silver halide photosensitive material, it is preferred that the concentration in coating composition of the fluorinated compound of the present invention be in the range of 0.003 to 0.5% by weight and, based on gelatin solid contents, 0.03 to 5% by weight.

In the present invention, at least one compound selected from the fluorinated compound represented by the general formula (A) and the fluorinated compound represented by the general formula (B) may be contained. A plurality of compounds selected from those represented by the general formula (A) alone, by the general formula (B) alone, or by both the general formula (A) and the general formula (B) may also be used in combination.

The substituent, T, as an example of substituents which may be possessed by groups capable of substitution in the above general formulas will be described below.

The substituent, T, can be, for example, any of an alkyl group (preferably having 1 to 20 carbon atoms, more preferably 1 to 12 carbon atoms and especially preferably 1 to 8 carbon atoms; e.g., methyl, ethyl, isopropyl, tert-butyl, n-octyl, n-decyl, n-hexadecyl, cyclopropyl, cyclopentyl or cyclohexyl), alkenyl group (preferably having 2 to 20 carbon atoms, more preferably 2 to 12 carbon atoms and especially preferably 2 to 8 carbon atoms; e.g., vinyl, allyl, 2-but enyl or 3-pentenyl), alkynyl group (preferably having 2 to 20 carbon atoms, more preferably 2 to 12 carbon atoms and especially preferably 2 to 8 carbon atoms; e.g., propargyl or 3-pentynyl), aryl group (preferably having 6 to 30 carbon atoms, more preferably 6 to 20 carbon atoms and especially preferably 6 to 12 carbon atoms; e.g., phenyl, p-methylphenyl or naphthyl), substituted or unsubstituted amino group (preferably having 0 to 20 carbon atoms, more preferably 0 to 10 carbon atoms and especially preferably 0 to 6 carbon atoms; e.g., unsubstituted amino, methylamino, dimethylamino, diethylamino or dibenzylamino), alkoxy group (preferably having 1 to 20 carbon atoms, more preferably 1 to 12 carbon atoms and especially preferably 1 to 8 carbon atoms; e.g., methoxy, ethoxy or butoxy), aryloxy group (preferably having 6 to 20 carbon atoms, more preferably 6 to 16 carbon atoms and especially preferably 6 to 12 carbon atoms; e.g., phenoxy or 2-naphthoxy), acyl

group (preferably having 1 to 20 carbon atoms, more preferably 1 to 16 carbon atoms and especially preferably 1 to 12 carbon atoms; e.g., acetyl, benzoyl, formyl or pivaloyl), alkoxy carbonyl group (preferably having 2 to 20 carbon atoms, more preferably 2 to 16 carbon atoms and especially preferably 2 to 12 carbon atoms; e.g., methoxycarbonyl or ethoxycarbonyl), aryloxy carbonyl group (preferably having 7 to 20 carbon atoms, more preferably 7 to 16 carbon atoms and especially preferably 7 to 10 carbon atoms; e.g., phenoxy carbonyl), acyloxy group (preferably having 2 to 20 carbon atoms, more preferably 2 to 16 carbon atoms and especially preferably 2 to 10 carbon atoms; e.g., acetoxy or benzyloxy), acylamino group (preferably having 2 to 20 carbon atoms, more preferably 2 to 16 carbon atoms and especially preferably 2 to 10 carbon atoms; e.g., acetyl amino or benzoyl amino), alkoxy carbonyl amino group (preferably having 2 to 20 carbon atoms, more preferably 2 to 16 carbon atoms and especially preferably 2 to 12 carbon atoms; e.g., methoxycarbonyl amino), aryloxy carbonyl amino group (preferably having 7 to 20 carbon atoms, more preferably 7 to 16 carbon atoms and especially preferably 7 to 12 carbon atoms; e.g., phenoxy carbonyl amino), sulfonyl amino group (preferably having 1 to 20 carbon atoms, more preferably 1 to 16 carbon atoms and especially preferably 1 to 12 carbon atoms; e.g., methanesulfonyl amino or benzene sulfonyl amino), sulfamoyl group (preferably having 0 to 20 carbon atoms, more preferably 0 to 16 carbon atoms and especially preferably 0 to 12 carbon atoms; e.g., sulfamoyl, methylsulfamoyl, dimethylsulfamoyl or phenylsulfamoyl), carbamoyl group (preferably having 1 to 20 carbon atoms, more preferably 1 to 16 carbon atoms and especially preferably 1 to 12 carbon atoms; e.g., unsubstituted carbamoyl, methylcarbamoyl, diethylcarbamoyl or phenylcarbamoyl), alkylthio group (preferably having 1 to 20 carbon atoms, more preferably 1 to 16 carbon atoms and especially preferably 1 to 12 carbon atoms; e.g., methylthio or ethylthio), arylthio group (preferably having 6 to 20 carbon atoms, more preferably 6 to 16 carbon atoms and especially preferably 6 to 12 carbon atoms; e.g., phenylthio), sulfonyl group (preferably having 1 to 20 carbon atoms, more preferably 1 to 16 carbon atoms and especially preferably 1 to 12 carbon atoms; e.g., mesyl or tosyl), sulfinyl group (preferably having 1 to 20 carbon atoms, more preferably 1 to 16 carbon atoms and especially preferably 1 to 12 carbon atoms; e.g., methanesulfinyl or benzenesulfinyl), ureido group (preferably having 1 to 20 carbon atoms, more preferably 1 to 16 carbon atoms and especially preferably 1 to 12 carbon atoms; e.g., unsubstituted ureido, methylureido or phenylureido), phosphoramido group (preferably having 1 to 20 carbon atoms, more preferably 1 to 16 carbon atoms and especially preferably 1 to 12 carbon atoms; e.g., diethylphosphoramido or phenylphosphoramido), hydroxyl group, mercapto group, halogen atom (e.g., fluorine atom, chlorine atom, bromine atom or iodine atom), cyano group, sulfo group, carboxyl group, nitro group, hydroxamic acid group, sulfino group, hydrazino group, imino group, heterocyclic group (preferably having 1 to 30 carbon atoms, more preferably 1 to 12 carbon atoms, and containing a heteroatom such as a nitrogen atom, an oxygen atom or a sulfur atom; e.g., imidazolyl, pyridyl, quinolyl, furyl, piperidyl, morpholino, benzoxazolyl, benzimidazolyl or benzthiazolyl) and silyl group (preferably having 3 to 40 carbon atoms, more preferably 3 to 30 carbon atoms and especially preferably 3 to 24 carbon atoms; e.g., trimethylsilyl or triphenylsilyl). These substituents may have further substituents. In the use of two or more substituents, they may be identical.

with or different from each other. Moreover, if appropriate, the substituents may bond together to form a ring.

It is preferred that the silver halide emulsion for use in the photosensitive material of the present invention be a silver iodobromide, silver bromide or silver chloroiodobromide tabular grain emulsion.

With respect to the color photosensitive material of the present invention, preferably, each unit light-sensitive layer is constituted of multiple silver halide emulsion layers which exhibit substantially identical color sensitivity but are different in speed. Further, 50% or more of the total projected area of silver halide grains contained in at least one layer of the emulsion layers with the highest photographic speed among the silver halide emulsion layers constituting each of the unit light-sensitive layers consists of tabular silver halide grains (hereinafter also referred to as "tabular grains"). In the present invention, the average aspect ratio of such tabular grains is preferably 8 or higher, more preferably 12 or higher, and most preferably 15 or higher.

With respect to tabular grains, the aspect ratio refers to the ratio of diameter to thickness of silver halides. That is, the aspect ratio is the quotient of diameter divided by thickness with respect to each individual silver halide grain. Herein, the diameter refers to the diameter of a circle with an area equal to the projected area of grain exhibited when silver halide grains are observed through a microscope or an electron microscope. Further, herein, the average aspect ratio refers to the average of aspect ratios regarding all the tabular grains of each emulsion.

The method of taking a transmission electron micrograph by the replica technique and determining the equivalent circle diameter and thickness of each individual grain can be mentioned as an example of aspect ratio determining method. In the mentioned method, the thickness is calculated from the length of replica shadow.

The configuration of tabular grains of the present invention is generally hexagonal. The terminology "hexagonal configuration" means that the shape of the main plane of tabular grains is hexagonal, the neighboring side ratio (maximum side length/minimum side length) thereof being 2 or less. The neighboring side ratio is preferably 1.6 or less, more preferably 1.2 or less. That the lower limit thereof is 1.0 is needless to mention. In the grains of high aspect ratio, especially, triangular tabular grains are increased in the tabular grains. The triangular tabular grains are produced when the Ostwald ripening has excessively been advanced. From the viewpoint of obtaining substantially hexagonal tabular grains, it is preferred that the period of this ripening be minimized. For this purpose, it is requisite to endeavor to raise the tabular grain ratio by nucleation. It is preferred that one or both of an aqueous silver ion solution and an aqueous bromide ion solution contain gelatin for the purpose of raising the probability of occurrence of hexagonal tabular grains at the time of adding silver ions and bromide ions to a reaction mixture according to the double jet technique, as described in JP-A-63-11928 by Saito.

The hexagonal tabular grains for use in the present invention are formed through the steps of nucleation, Ostwald ripening and growth. Although all of these steps are important for suppressing the spread of grain size distribution, especial attention should be paid so as to prevent the spread of size distribution at the first nucleation step because the spread of size distribution brought about in a previous step cannot be narrowed by an ensuing step. What is important in the nucleation step is the relationship between the temperature of reaction mixture and the period of nucleation comprising adding silver ions and bromide ions

to a reaction mixture according to the double jet technique and producing precipitates. JP-A-63-92942 by Saito describes that it is preferred that the temperature of the reaction mixture at the time of nucleation be in the range of from 20 to 45° C. for realizing a monodispersity enhancement. Further, JP-A-2-222940 by Zola et al describes that the suitable temperature at nucleation is 60° C. or below.

In order to obtain monodisperse tabular grains with high aspect ratio, gelatin is additionally added during grain formation. At this time, the gelatin use is preferably chemically modified gelatin described in JP-A's 10-148897 and 11-143002. The chemically modified gelatin is one characterized in that at the time of chemically modifying amino groups thereof, at least two carboxyl groups are introduced. Trimellitated gelatin is preferably used. Succinated gelatin is also preferable. The gelatin is preferably added before growth step, and more preferably added immediately after nucleation. The addition amount is preferably 60% or more, more preferably 80% or more, and especially preferably 90% or more to the total weight of dispersing medium during grain formation.

Tabular grain emulsion preferably comprises silver iodobromide or silver chloroiodobromide. Although silver chloride may be contained, the silver chloride content is preferably 8 mol % or less, more preferably 3 mol % or less, and most preferably 0 mol %. For silver iodide content, since the coefficient variation of grain size distribution of the tabular grain emulsion is preferably 30% or less, the silver iodide content is preferably 20 mol % or less. It becomes easier to reduce the variation coefficient of distribution of equivalent circle diameters of the tabular grain emulsion by reducing the silver iodide content. Especially, the coefficient variation of the distribution of grain sizes of the tabular grain emulsion is preferably 20% or less, and the silver iodide content is preferably 10 mol % or less.

The tabular grain emulsion preferably has an intra grain structure of silver iodide distribution. In this case, the structure of the silver iodide distribution may be a double structure, a triple structure, a quadruple structure, or higher structures.

In the present invention, the tabular grains preferably have dislocation lines. The dislocation lines of the tabular grains can be observed by the direct method using a transmission electron microscope at low temperatures as described in, for example, J. F. Hamilton, Phot. Sci. Eng., 11, 57 (1967) and T. Shiozawa, J. Soc. Phot. Sci. Japan, 3, 5, 213 (1972). Illustratively, silver halide grains are harvested from the emulsion with the care that the grains are not pressurized with such a force that dislocation lines occur on the grains, are put on a mesh for electron microscope observation and, while cooling the specimen so as to prevent damaging (printout, etc.) by electron beams, are observed by the transmission method. The greater the thickness of the above grains, the more difficult the transmission of electron beams. Therefore, the use of an electron microscope of high voltage type (at least 200 KV on the grains of 0.25 µm in thickness) is preferred for ensuring clearer observation. The thus obtained photograph of grains enables determining the position and number of dislocation lines in each grain viewed in the direction perpendicular to the main planes.

In the emulsion of the present invention the number of dislocation lines of the tabular grains is preferably at least 10 per grain on the average and more preferably at least 20 per grain on the average. When dislocation lines are densely present or when dislocation lines are observed in the state of crossing each other, it happens that the number of dislocation lines per grain cannot accurately be counted. However,

in this instance as well, rough counting on the order of, for example, 10, 20 or 30 dislocation lines can be effected, so that a clear distinction can be made from the presence of only a few dislocation lines. The average number of dislocation lines per grain is determined by counting the number of dislocation lines of each of at least 100 grains and calculating a number average thereof. There are instances when hundreds of dislocation lines are observed.

Dislocation lines can be introduced in, for example, the vicinity of the periphery of tabular grains. In this instance, the dislocation is nearly perpendicular to the periphery, and each dislocation line extends from a position corresponding to x % of the distance from the center of tabular grains to the side (periphery) to the periphery. The value of x preferably ranges from 10 to less than 100, more preferably from 30 to less than 99, and most preferably from 50 to less than 98. In this instance, the figure created by binding the positions from which the dislocation lines start is nearly similar to the configuration of the grain. The created figure may be one which is not a complete similar figure but deviated. The dislocation lines of this type are not observed around the center of the grain. The dislocation lines are crystallographically oriented approximately in the (211) direction. However, the dislocation lines often meander and may also cross each other.

Dislocation lines may be positioned either nearly uniformly over the entire zone of the periphery of the tabular grains or local points of the periphery. That is, referring to, for example, hexagonal tabular silver halide grains, dislocation lines may be localized either only in the vicinity of six apexes or only in the vicinity of one of the apexes. Contrarily, dislocation lines can be localized only in the sides excluding the vicinity of six apexes.

Furthermore, dislocation lines may be formed over regions including the centers of two mutually parallel main planes of tabular grains. In the case where dislocation lines are formed over the entire regions of the main planes, the dislocation lines may crystallographically be oriented approximately in the (211) direction when viewed in the direction perpendicular to the main planes, and the formation of the dislocation lines may be effected either in the (110) direction or randomly. Further, the length of each dislocation line may be random, and the dislocation lines may be observed as short lines on the main planes or as long lines extending to the side (periphery). The dislocation lines may be straight or often meander. In many instances, the dislocation lines cross each other.

The position of dislocation lines may be localized on the periphery, or on main planes or local points thereof as mentioned above, or the formation of dislocation lines may be effected on a combination thereof. That is, dislocation lines may be concurrently present on both the periphery and the main planes.

The introduction of dislocation lines in the tabular grains can be accomplished by disposing a specified phase of high silver iodide content within the grains. In the dislocation line introduction, the phase of high silver iodide content may be provided with discontinuous regions of high silver iodide content. Practically, the phase of high silver iodide content within the grains can be obtained by first preparing base grains, providing them with a phase of high silver iodide content and covering the outside thereof with a phase of silver iodide content lower than that of the phase of high silver iodide content. The silver iodide content of the base tabular grains is lower than that of the phase of high silver iodide content, and is preferably 0 to 20 mol %, more preferably 0 to 15 mol %.

In the present invention, the terminology "phase of high silver iodide content within the grains" refers to a silver halide solid solution containing silver iodide. The silver halide of this solid solution is preferably silver iodide, silver iodobromide or silver chloroiodobromide, more preferably silver iodide or silver iodobromide (the silver iodide content is in the range of 10 to 40 mol % based on the silver halides contained in the phase of high silver iodide content). For selectively causing the phase of high silver iodide content within the grains (hereinafter referred to as "internal high silver iodide phase") to be present on any place of the sides, corners and faces of the base grains, it is desirable to control forming conditions for the base grains, forming conditions for the internal high silver iodide phase and forming conditions for the phase covering the outside thereof. With respect to the forming conditions for the base grains, the pAg (logarithm of inverse number of silver ion concentration), the presence or absence, type and amount of silver halide solvent and the temperature are important factors.

Regulating the pAg at base grain growth to 8.5 or less, preferably 8 or less, enables selectively causing the internal high silver iodide phase to be present near the apex or on the face of the base grains in the subsequent step of forming the internal high silver iodide phase.

On the other hand, regulating the pAg at base grain growth to at least 8.5, preferably at least 9, enables causing the internal high silver iodide phase to be present on the side of the base grains in the subsequent step of forming the internal high silver iodide phase. The threshold value of the pAg is changed upward or downward depending on the temperature and the presence or absence, type and amount of silver halide solvent. When, for example, a thiocyanate is used as the silver halide solvent, the threshold value of the pAg is deviated toward a higher value. What is most important as the pAg at growth is the pAg at the termination of growth of base grains. On the other hand, even when the pAg at growth does not satisfy the above value, the selected position of the internal high silver iodide phase can be controlled by carrying out, after the growth of base grains, the regulation to the above pAg and a ripening. Ammonia, an amine compound, a thiourea derivative or a thiocyanate salt is effective as the silver halide solvent. For the formation of the internal high silver iodide phase, use can be made of the so-called conversion methods.

These conversion methods include one in which, during grain formation, halide ions whose salts formed with silver ions exhibit a solubility lower than that of the salts formed with the halide ions that are forming the grains or the vicinity of the surface of the grains occurring at the time of grain formation, are added. In the present invention, it is preferred that the amount of added low-solubility halide ions be at least some value (relating to halogen composition) relative to the surface area of grains occurring at the time of the addition. For example, it is preferred that, during grain formation, KI be added in an amount not smaller than some amount relative to the surface area of silver halide grains occurring at the time of the grain formation. Specifically, it is preferred that an iodide salt be added in an amount of at least  $8.2 \times 10^{-5}$  mol/m<sup>2</sup>.

Preferred process for forming the internal high silver iodide phase comprises adding an aqueous solution of a silver salt simultaneously with the addition of an aqueous solution of halide salts containing an iodide salt.

For example, an aqueous solution of AgNO<sub>3</sub> is added simultaneously with the addition of an aqueous solution of KI by the double jet. The addition initiating times and addition completing times of the aqueous solution of KI and

the aqueous solution of  $\text{AgNO}_3$  may be differed from each other, that is, the one may be earlier or later than the other. The addition molar ratio of an aqueous solution of  $\text{AgNO}_3$  to an aqueous solution of  $\text{KI}$  is preferably at least 0.1, more preferably at least 0.5, and most preferably at least 1. The total addition molar amount of an aqueous solution of  $\text{AgNO}_3$  relative to halide ions within the system and added iodide ions may fall in a silver excess region. It is preferred that the  $\text{pAg}$  exhibited when the aqueous solution of halide containing such iodide ions and the aqueous solution of silver salt are added by the double jet be decreased in accordance with the passage of double jet addition time. The  $\text{pAg}$  prior to the addition initiation is preferably in the range of 6.5 to 13, more preferably 7.0 to 11. The  $\text{pAg}$  at the time of addition completion is most preferably in the range of 6.5 to 10.0.

In the performing of the above process, it is preferred that the solubility in the mixture system be as low as possible. Accordingly, the temperature of the mixture system exhibited at the time of formation of the high silver iodide phase is preferably in the range of 30 to 80° C., more preferably 30 to 70° C.

Furthermore, the formation of the internal high silver iodide phase can preferably be performed by adding fine grains of silver iodide, fine grains of silver iodobromide, fine grains of silver chloroiodide or fine grains of silver chloroiodobromide. It is especially preferred that the formation be effected by adding fine grains of silver iodide. Although these fine grains generally have a size of 0.01 to 0.1  $\mu\text{m}$ , use can also be made of fine grains with a size of not greater than 0.01  $\mu\text{m}$ , or 0.1  $\mu\text{m}$  or more. With respect to the process for preparing these fine grains of silver halide, reference can be made to descriptions of JP-A's-1-183417, 2-44335, 1-183644, 1-183645, 2-43534 and 2-43535. The internal high silver iodide phase can be provided by adding these fine grains of silver halide and conducting a ripening. When the fine grains are dissolved by ripening, use can be made of the aforementioned silver halide solvent. It is not needed that all these added fine grains be immediately dissolved and disappear. It is satisfactory if, when the final grains have been completed, they are dissolved and disappear.

The position of the internal high silver iodide phase, as measured from the center of, for example, a hexagon resulting from grain projection, is preferably present in the range of 5 to less than 100 mol %, more preferably 20 to less than 95 mol %, and most preferably 50 to less than 90 mol %, based on the amount of silver of the whole grain. The amount of silver halide forming this internal high silver iodide phase, in terms of the amount of silver, is 50 mol % or less, preferably 20 mol % or less, based on the amount of silver of the whole grain. With respect to the above high silver iodide phase, there are provided recipe values of the production of silver halide emulsion, not values obtained by measuring the halogen composition of final grains according to various analytical methods. The internal high silver iodide phase is often caused to completely disappear in final grains by, for example, recrystallization during the shell covering step, and all the above silver amounts relate to recipe values thereof.

Therefore, although the observation of dislocation lines can be easily performed in the final grains by the above method, the internal silver iodide phase introduced for the introduction of dislocation lines often cannot be confirmed as a clear phase because the boundary silver iodide composition is continuously changed. The halogen composition at each grain part can be determined by a combination of X-ray diffractometry, the EPMA method (also known as the XMA

method, in which silver halide grains are scanned by electron beams to thereby detect the silver halide composition), the ESCA method (also known as the XPS method, in which X rays are irradiated and photoelectrons emitted from grain surface are separated into spectra), etc.

The outside phase which covers the internal high silver iodide phase has a silver iodide content lower than that of the internal high silver iodide phase. The silver iodide content of the covering outside phase is preferably in the range of 0 to 10 mol %, more preferably 0 to 20 mol %, and most preferably 0 to 10 mol %, based on the silver halide contained in the covering outside phase.

Although the temperature and  $\text{pAg}$  employed at the formation of the outside phase which covers the internal high silver iodide phase are arbitrary, the temperature preferably ranges from 30 to 80° C., most preferably from 35 to 70° C., and the  $\text{pAg}$  preferably ranges from 6.5 to 11.5. The use of the aforementioned silver halide solvent is occasionally preferred, and the most preferred silver halide solvent is a thiocyanate salt.

Another method of introducing dislocation lines in the tabular grains comprises using an iodide ion-releasing agent as described in JP-A-6-11782, which can preferably be employed.

Also, dislocation lines can be introduced by appropriately combining this method of introducing dislocation lines with the aforementioned method of introducing dislocation lines.

The variation coefficient of the intergranular iodine distribution of silver halide grains for use in the present invention is preferably 20% or less, more preferably 15% or less, and much more preferably 10% or less. When the variation coefficient of the iodine content distribution of each silver halide is greater than 20%, unfavorably, a high contrast is not realized and a sensitivity lowering is intense when a pressure is applied.

Any known processes such as the process of adding fine grains as described, for example, in JP-A-1-183417 and the process of using an iodide ion-releasing agent as described in JP-A-2-68538 can be employed either individually or in combination for the production of silver halide grains whose intergranular iodine distribution is narrow for use in the present invention.

The silver halide grains for use in the present invention preferably have a variation coefficient of intergranular iodine distribution of 20% or less. The process described in JP-A-3-213845 can be used as the most suitable process for converting the intergranular iodine distribution to a monodispersion. That is, a monodisperse intergranular iodine distribution can be accomplished by a process in which fine silver halide grains containing silver iodide in an amount of at least 95 mol % are formed by mixing together an aqueous solution of a water soluble silver salt and an aqueous solution of a water soluble halide (containing at least 95 mol % of iodide ions) by means of a mixer provided outside a reactor vessel for crystal growth and, immediately after the formation, fed in the reactor vessel. The terminology "reactor vessel" used herein means the vessel in which the nucleation and/or crystal growth of tabular silver halide grains is carried out.

With respect to the above process of mixer preparation followed by adding procedure and the preparatory means for use therein, the following three techniques can be employed as described in JP-A-3-213845:

- (1) immediately after formation of fine grains in a mixer, the fine grains are transferred into a reactor vessel;
- (2) powerful and effective agitation is carried out in the mixer; and

(3) an aqueous solution of protective colloid is injected into the mixer.

The protective colloid used in technique (3) above may be separately injected in the mixer, or may be incorporated in the aqueous solution of silver halide or the aqueous solution of silver nitrate before the injection in the mixer. The concentration of protective colloid is at least 1% by weight, preferably in the range of 2 to 5% by weight. Examples of polymeric compounds exhibiting a protective colloid function to the silver halide grains for use in the present invention include polyacrylamide polymers, amino polymers, polymers having thioether groups, polyvinyl alcohol, acrylic polymers, hydroxyquinoline having polymers, cellulose, starch, acetal, polyvinylpyrrolidone and ternary polymers.

Low-molecular-weight gelatin can preferably be used as the above polymeric compound. The molecular weight of low-molecular-weight gelatin is preferably 30,000 or less, more preferably 10,000 or less.

The grain formation temperature in the preparation of fine silver halide grains is preferably 35° C. or below, more preferably 25° C. or below. The temperature of the reactor vessel in which fine silver halide grains are incorporated is at least 50° C., preferably at least 60° C., and more preferably at least 70° C.

The grain size of fine-size silver halide for use in the present invention can be determined by placing grains on a mesh and making a direct observation through a transmission electron microscope. The size of fine grains of the present invention is 0.3  $\mu$ m or less, preferably 0.1  $\mu$ m or less, and more preferably 0.01  $\mu$ m or less. This fine silver halide may be added simultaneously with the addition of other halide ions and silver ions, or may be separately added. The fine silver halide grains are mixed in an amount of 0.005 to 20 mol %, preferably 0.01 to 10 mol %, based on the total silver halide.

The silver iodide content of each individual grain can be measured by analyzing the composition of each individual grain by means of an X-ray microanalyzer. The terminology "variation coefficient of intergranular iodine distribution" means a value defined by the formula:

$$\text{variation coefficient} = (\text{standard deviation}/\text{av. silver iodide content}) \times 100$$

wherein the standard deviation, specifically the standard deviation of silver iodide content, and the average silver iodide content are obtained by measuring the silver iodide contents of at least 100, preferably at least 200, and more preferably at least 300 emulsion grains. The measuring of the silver iodide content of each individual grain is described in, for example, EP No. 147,868. There are cases in which a correlation exists between the silver iodide content  $Y_i$  (mol %) of each individual grain and the equivalent spherical diameter  $X_i$  ( $\mu$ m) of each individual grain and cases in which no such correlation exists. It is preferred that no correlation exist therebetween. The structure associated with the silver halide composition of grains of the present invention can be identified by, for example, a combination of X-ray diffractometry, the EPMA method (also known as the XMA method, in which silver halide grains are scanned by electron beams to thereby detect the silver halide composition) and the ESCA method (also known as the XPS method, in which X rays are irradiated and photoelectrons emitted from grain surface are separated into spectra). In the measuring of silver iodide content in the present invention, the terminology "grain surface" refers to the region whose depth from

surface is about 5 nm, and the terminology "grain internal part" refers to the region other than the above surface. The halogen composition of such a grain surface can generally be measured by the ESCA method.

5 In the present invention, use can be made of not only the above tabular grains but also regular crystal grains such as cubic, octahedral and tetradecahedral grains and, further, irregular twinned crystal grains.

Selenium sensitization or gold sensitization is preferably 10 performed on the silver halide emulsion of the present invention.

Selenium compounds disclosed in hitherto published 15 patents can be used as the selenium sensitizer in the present invention. In the use of labile selenium compound and/or nonlabile selenium compound, generally, it is added to an emulsion and the emulsion is agitated at high temperature, preferably 40° C. or above, for a given period of time. Compounds described in, for example, Jpn. Pat. Appln. KOKOKU Publication No. (hereinafter referred to as JP-B-) 20 44-15748, JP-B-43-13489, JP-A's-4-25832 and 4-109240 are preferably used as the labile selenium compound.

Specific examples of the labile selenium sensitizers 25 include isoselenocyanates (for example, aliphatic isoselenocyanates such as allyl isoselenocyanate), selenoureas, selenoketones, selenoamides, selenocarboxylic acids (for example, 2-selenopropionic acid and 2-selenobutyric acid), selenoesters, diacyl selenides (for example, bis(3-chloro-2, 6-dimethoxybenzoyl) selenide), selenophosphates, phosphine selenides and colloidal metal selenium.

30 The labile selenium compounds, although preferred types thereof are as mentioned above, are not limited thereto. It is generally understood by persons of ordinary skill in the art to which the invention pertains that the structure of the labile selenium compound as a photographic emulsion sensitizer is not so important as long as the selenium is labile and that the labile selenium compound plays no other role than having its selenium carried by organic portions of selenium sensitizer molecules and causing it to present in labile form in the emulsion. In the present invention, the labile selenium compounds of this broad concept can be used advantageously.

35 Compounds described in JP-B's-46-4553, 52-34492 and 52-34491 can be used as the nonlabile selenium compound in the present invention. Examples of the nonlabile selenium 40 compounds include selenious acid, potassium selenocyanate, selenazoles, quaternary selenazole salts, diaryl selenides, diaryl diselenides, dialkyl selenides, dialkyl diselenides, 2-selenazolidinedione, 2-selenoxazolidinethione and derivatives thereof.

45 These selenium sensitizers are dissolved in water or an organic solvent such as methanol and ethanol or a mixed solvent of these, and added at the time of chemical sensitization. Preferably, the addition is performed prior to the initiation of chemical sensitization. The above selenium 50 sensitizers can be used either individually or in combination. The joint use of an labile selenium compound and a non-labile selenium compound is preferred.

55 The addition amount of selenium sensitizer for use in the present invention, although varied depending on the activity of employed selenium sensitizer, the type and size of silver halide, the ripening temperature and time, etc., is preferably in the range of  $2 \times 10^{-6}$  to  $5 \times 10^{-6}$  mol per mol of silver halide. The temperature of chemical sensitization in the use of a selenium sensitizer is preferably between 40° C. and 80° C. The pAg and pH are arbitrary. For example, with respect to pH, the effect of the present invention can be exerted even if it widely ranges from 4 to 9.

Selenium sensitization is effectively attained in the presence of a silver halide solvent.

Examples of the silver halide solvent usable in the present invention are (a) organic thioethers described in, e.g., U.S. Pat. Nos. 3,271,157, 3,531,289, and 3,574,628, and JP-A's 54-1019 and 54-158917, (b) thiourea derivatives described in, e.g., JP-A's-53-82408, 55-77737, and 55-2982, (c) a silver halide solvent having a thiocarbonyl group sandwiched between an oxygen or sulfur atom and a nitrogen atom described in JP-A-53-144319, (d) imidazoles described in JP-A-54-100717, (e) ammonia, and (f) thiocyanate.

Particularly preferable solvents are thiocyanate, ammonia, and tetramethylthiourea. Although the amount of a solvent used changes in accordance with the type of the solvent, a preferable amount of, e.g., thiocyanate is  $1 \times 10^{-4}$  to  $1 \times 10^{-2}$  mol per mol of a silver halide.

The oxidation number of gold of the gold sensitizer mentioned above may be either +1 or +3, and gold compounds customarily used as gold sensitizers can be employed. Representative examples thereof include chloroauric acid salts, potassium chloroaurate, auric trichloride, potassium auric thiocyanate, potassium iodoaurate, tetracyanoauric acid, ammonium aurothiocyanate, pyridyltrichlorogold, gold sulfide and gold selenide. The addition amount of gold sensitizer, although varied depending on various conditions, is preferably between  $1 \times 10^{-7}$  mol and  $5 \times 10^{-5}$  mol per mol of silver halide as a yardstick.

With respect to the emulsion for use in the present invention, it is desired to perform sulfur sensitization in combination for the chemical sensitization.

The sulfur sensitization is generally performed by adding a sulfur sensitizer and agitating the emulsion at high temperature, preferably 40° C. or above, for a given period of time.

In the above sulfur sensitization, those known as sulfur sensitizers can be used. For example, use can be made of thiosulfates, allylthiocarbamidothiourea, allyl isothiacyanate, cystine, p-toluenethiosulfonates and rhodanine. Use can also be made of other sulfur sensitizers described in, for example, U.S. Pat. Nos. 1,574,944, 2,410,689, 2,278,947, 2,728,668, 3,501,313 and 3,656,955, West German Patent No. 1,422,869, JP-B-56-24937 and JP-A-55-45016. The addition amount of sulfur sensitizer is satisfactory if it is sufficient to effectively increase the sensitivity of the emulsion. This amount, although varied to a large extent under various conditions such as the pH, temperature and size of silver halide grains, is preferably in the range of  $1 \times 10^{-7}$  to  $5 \times 10^{-5}$  mol per mol of silver halide.

The silver halide emulsion for use in the present invention can be subjected to a reduction sensitization during the grain formation, or after the grain formation but before the chemical sensitization, during the chemical sensitization or after the chemical sensitization.

The reduction sensitization can be performed by a method selected from among the method in which a reduction sensitizer is added to the silver halide emulsion, the method commonly known as silver ripening in which growth or ripening is carried out in an environment of pAg as low as 1 to 7 and the method commonly known as high-pH ripening in which growth or ripening is carried out in an environment of pH as high as 8 to 11. At least two of these methods can be used in combination.

The above method in which a reduction sensitizer is added is preferred from the viewpoint that the level of reduction sensitization can be finely regulated.

Examples of known reduction sensitizers include stannous salts, ascorbic acid and derivatives thereof, amines and polyamino acids, hydrazine derivatives, formamidine-sulfonic acid, silane compounds and borane compounds. In the reduction sensitization employed in the present invention, appropriate one may be selected from among these known reduction sensitizers and used or at least two may be selected and used in combination. Preferred reduction sensitizers are stannous chloride, thiourea dioxide, dimethylaminoborane, ascorbic acid and derivatives thereof. Although the addition amount of reduction sensitizer must be selected because it depends on the emulsion manufacturing conditions, it is preferred that the addition amount range from  $10^{-7}$  to  $10^{-3}$  mol per mol of silver halide.

Each reduction sensitizer is dissolved in water or any of organic solvents such as alcohols, glycols, ketones, esters and amides and added during the grain growth. Although the reduction sensitizer may be put in a reaction vessel in advance, it is preferred that the addition be effected at an appropriate time during the grain growth. It is also suitable to add in advance the reduction sensitizer to an aqueous solution of a water-soluble silver salt or a water-soluble alkali halide and to precipitate silver halide grains with the use of the resultant aqueous solution. Alternatively, the reduction sensitizer solution may preferably be either divided and added a plurality of times in accordance with the grain growth or continuously added over a prolonged period of time.

An oxidizer capable of oxidizing silver is preferably used during the process of producing the emulsion for use in the present invention. The silver oxidizer is a compound having an effect of acting on metallic silver to thereby convert the same to silver ion. A particularly effective compound is one that converts very fine silver grains, formed as a by-product in the step of forming silver halide grains and the step of chemical sensitization, into silver ions. Each silver ion produced may form a silver salt sparingly soluble in water, such as a silver halide, silver sulfide or silver selenide, or may form a silver salt easily soluble in water, such as silver nitrate. The silver oxidizer may be either an inorganic or an organic substance. Examples of suitable inorganic oxidizers include ozone, hydrogen peroxide and its adducts (e.g.,  $\text{NaBO}_2 \cdot \text{H}_2\text{O}_2 \cdot 3\text{H}_2\text{O}_2$ ,  $2\text{NaCO}_3 \cdot 3\text{H}_2\text{O}_2$ ,  $\text{Na}_4\text{P}_2\text{O}_7 \cdot 2\text{H}_2\text{O}_2$  and  $2\text{Na}_2\text{SO}_4 \cdot \text{H}_2\text{O}_2 \cdot 2\text{H}_2\text{O}$ ), peroxy acid salts (e.g.,  $\text{K}_2\text{S}_2\text{O}_8$ ,  $\text{K}_2\text{C}_2\text{O}_4$  and  $\text{K}_2\text{P}_2\text{O}_8$ ), peroxy complex compounds (e.g.,  $\text{K}_2[\text{Ti}(\text{O}_2)\text{C}_2\text{O}_4] \cdot 3\text{H}_2\text{O}$ ,  $4\text{K}_2\text{SO}_4 \cdot \text{Ti}(\text{O}_2)\text{OH} \cdot \text{SO}_4 \cdot 2\text{H}_2\text{O}$  and  $\text{Na}_3[\text{VO}(\text{O}_2)(\text{C}_2\text{H}_4)_2] \cdot 6\text{H}_2\text{O}$ ), permanganates (e.g.,  $\text{KMnO}_4$ ), chromates (e.g.,  $\text{K}_2\text{Cr}_2\text{O}_7$ ) and other oxyacid salts, halogen elements such as iodine and bromine, perhalogenates (e.g., potassium periodate), salts of high-valence metals (e.g., potassium hexacyanoferrate (II)) and thiosulfonates.

Examples of suitable organic oxidizers include quinones such as p-quinone, organic peroxides such as peracetic acid and perbenzoic acid and active halogen releasing compounds (e.g., N-bromosuccinimide, chloramine T and chloramine B).

Oxidizers preferred in the present invention are inorganic oxidizers selected from among ozone, hydrogen peroxide and its adducts, halogen elements and thiosulfonates and organic oxidizers selected from among quinones.

The use of the silver oxidizer in combination with the above reduction sensitization is preferred. This combined use can be effected by performing the reduction sensitization after the use of the oxidizer or vice versa or by simultaneously performing the reduction sensitization and the use

of the oxidizer. These methods can be performed during the step of grain formation or the step of chemical sensitization.

The photographic emulsion of the present invention can exhibit excellent color saturation by spectrally sensitizing preferably by methine dyes and other dyes. The dyes to be used include a cyanine dye, merocyanine dye, complex cyanine dye, complex merocyanine dye, holopolar cyanine dyes, hemicyanine dye, styryl dye, and hemioxonol dye. Especially useful dyes are those that belong to a cyanine dye, merocyanine dye, and complex merocyanine dye. Any of nuclei commonly used in cyanine dyes as basic heterocyclic nuclei can be applied to these dyes. Examples of such applicable nuclei include a pyrrolidine nucleus, an oxazoline nucleus, a thiazoline nucleus, a pyrrole nucleus, an oxazole nucleus, a thiazole nucleus, a selenazole nucleus, an imidazole nucleus, a tetrazole nucleus and a pyridine nucleus; nuclei comprising these nuclei fused with alicyclic hydrocarbon rings; and nuclei comprising these nuclei fused with aromatic hydrocarbon rings, such as an indolenine nucleus, a benzindolenine nucleus, an indole nucleus, a benzoxazole nucleus, a naphthoxazole nucleus, a benzothiazole nucleus, a naphthothiazole nucleus, a benzoselenazole nucleus, a benzimidazole nucleus and a quinoline nucleus. These nuclei may have a carbon atom being substituted.

In the merocyanine dyes and composite merocyanine dyes, any of 5 or 6-membered heterocyclic nuclei such as a pyrazolin-5-one nucleus, a thiohydantoin nucleus, a 2-thioxazolidine-2,4-dione nucleus, a thiazolidine-2,4-dione nucleus, a rhodanine nucleus and a thiobarbituric acid nucleus can be applied as a nucleus having a ketomethylene structure.

These spectral sensitizing dyes may be used either individually or in combination. The spectral sensitizing dyes are often used in combination for the purpose of attaining supersensitization. Representative examples thereof are described in U.S. Pat. Nos. 2,688,545, 2,977,229, 3,397,060, 3,522,052, 3,527,641, 3,617,293, 3,628,964, 3,666,480, 3,672,898, 3,679,428, 3,703,377, 3,769,301, 3,814,609, 3,837,862 and 4,026,707, GB's 1,344,281 and 1,507,803, JP-B-43-4936 and 53-12375 and JP-A-52-110618 and 52-109925. The emulsion used in the present invention may contain a dye which itself exerts no spectral sensitizing effect or a substance which absorbs substantially none of visible radiation and exhibits supersensitization, together with the above spectral sensitizing dye.

Further, it is preferable to use a technique of improving light absorption ratio with a spectral sensitizing dye in combination with the present invention. For example, there can be mentioned a method in which a dye is adsorbed on the surface of silver halide grain in an amount of more than a single layer saturated adsorption (i.e., one layer adsorption) by using intermolecular force, or a method in which a compound consisting of a plurality of dye chromophores, so to called a linked dye, is adsorbed on a silver halide grain. Among these, the techniques described in the following patent applications are preferably used in combination with the present invention.

The publications and specifications of JP-A's 10-239789, 11-133531, 2000-267216, 2000-275772, 2001-75222, 2001-75247, 2001-75221, 2001-75226, 2001-75223, 2001-255615, 2002-23294, 10-171058, 10-186559, 10-197980, 2000-81678, 2001-5132, 2001-166413, 2002-49113, 64-91134, 10-110107, 10-171058, 10-226758, 10-307358, 10-307359, 10-310715, 2000-231174, 2000-231172, 2000-231173, and 2001-356442, and EP's 0985965A, 0985964A, 0985966A, 0985967A, 1085372A, 1085373A, 1172688A, 1199595A and 887700A1.

Further, it is preferable to use the techniques described in the publications of JP-A's 10-239789, 2001-75222 and 10-171058 in combination.

The addition timing of the spectral sensitizing dye to the emulsion may be performed at any stage of the process for preparing the emulsion which is known as being useful. Although the doping is most usually conducted at a stage between the completion of the chemical sensitization and the coating, the spectral sensitizing dye can be added simultaneously with the chemical sensitizer to thereby simultaneously effect the spectral sensitization and the chemical sensitization as described in U.S. Pat. Nos. 3,628,969 and 4,225,666. Alternatively, the spectral sensitization can be conducted prior to the chemical sensitization and, also, the spectral sensitizing dye can be added prior to the completion of silver halide grain precipitation to thereby initiate the spectral sensitization as described in JP-A-58-113928. Further, the above sensitizing dye can be divided prior to addition, that is, part of the sensitizing dye can be added prior to the chemical sensitization with the rest of the sensitizing dye added after the chemical sensitization as taught in U.S. Pat. No. 4,225,666. Still further, the spectral sensitizing dye can be added at any stage during the formation of silver halide grains according to the method disclosed in U.S. Pat. No. 4,183,756 and other methods.

When a plurality of sensitizing dyes are added a suitable method may be selected depending on the selected type of the sensitizing dye and desired spectral sensitivity, for example, from a method of adding each one separately with intervals, a method of adding them as a mixture, a method of adding one kind of sensitizing dye from a group of sensitizing dyes precedentially and adding the remaining dyes as a mixture with other sensitizing dyes.

The addition amount of the sensitizing dye may be from 35  $4 \times 10^{-6}$  to  $8 \times 10^{-3}$  mol per mol of silver halide. For preferable silver halide grains having a size of 0.2 to 1.2  $\mu\text{m}$ , about  $5 \times 10^{-5}$  to  $2 \times 10^{-3}$  mol per mol of silver is preferable.

Silver halide grains of the present invention has a twin plane distance of preferably 0.017  $\mu\text{m}$  or less. More preferably, the twin plane distance is 0.007 to 0.017  $\mu\text{m}$ , and especially preferably 0.007 to 0.015  $\mu\text{m}$ .

The fogging during aging of the silver halide emulsion for use in the present invention can be improved by adding and dissolving a previously prepared silver iodobromide emulsion at the time of chemical sensitization. Although the timing of the addition is arbitrary as long as it is performed during chemical sensitization, it is preferred that the silver iodobromide emulsion be first added and dissolved and, thereafter, a sensitizing dye and a chemical sensitizer be added in this order. The employed silver iodobromide emulsion has an iodine content lower than the surface iodine content of host grains, which is preferably a pure silver bromide emulsion. This silver iodobromide emulsion, although the size thereof is not limited as long as it is completely dissolvable, preferably has an equivalent spherical diameter of 0.1  $\mu\text{m}$  or less, more preferably 0.05  $\mu\text{m}$  or less. Although the addition amount of silver iodobromide emulsion depends on employed host grains, basically, it preferably ranges from 0.005 to 5 mol %, more preferably from 0.1 to 1 mol %, based on the mole of silver.

The emulsion used in the present invention may use a conventional dopant that is known to be useful for a silver halide emulsion. Examples of the conventional dopant are Fe, Co, Ni, Ru, Rh, Pd, Re, Os, Ir, Pt, Au, Hg, Pb, and Tl. In the present invention, hexacyano iron(II) complex, an hexacyano lutetium complexes (hereinafter simply referred to as "metal complex") are preferably used.

The addition amount of the metal complex is preferably  $10^{-7}$  mol or more but  $10^{-3}$  mol or less per mol of silver halide, and more preferably  $1.0 \times 10^{-5}$  mol or more but  $5 \times 10^{-4}$  mol per mol of silver halide.

The metal complex used in the present invention may be added at any stage of the preparation of silver halide grains, such as during nucleation, growth, physical ripening, and before and after chemical sensitization. The metal complex may also be added in several times in a separate matter. However, 50% or more of the metal complex contained in a silver halide grain are preferably contained within the layer of 1/2, in terms of silver amount, from the outermost surface of the silver halide grain. A layer containing no metal complex may be provided at outer position from a support than a layer containing a metal complex mentioned above.

It is preferable for these metal complexes to dissolve into water or a suitable solvent, and add directly to a reaction solution during the formation of silver halide grains, or to add into an aqueous solution of halide or aqueous solution of silver salt for forming silver halide grains, or to add into a solution other than these, and then use the solutions to grain formation, thereby incorporating the metal complex into the silver halide grains. Further, it is also preferable to add and dissolve silver halide fine grains to which a metal complex is previously contained, and deposit them on other silver halide grains, thereby incorporation the metal complex into the silver halide grains.

The hydrogen ion concentration in the reaction solution at the addition of these metal complexes is preferably pH of 1 to 10, and more preferably pH of 3 to 7.

The silver halide color photosensitive material of the present invention may have at least one each of a red-sensitive silver halide emulsion layer, a green-sensitive silver halide emulsion layer, a blue-sensitive emulsion layer and a non-light-sensitive layer on a support. When each of the emulsion layers is composed of two or more sub-layers having substantially the same color sensitivity but different in speed, it is preferable that a highest-speed emulsion layer of one of the color-sensitive layers does not substantially contain a DIR compound capable of releasing a development inhibitor and/or a precursor of a development inhibitor.

With respect to a multi-layered silver halide color photosensitive material, the arrangement of unit light-sensitive layers is generally, from the side nearer to a support, a red-sensitive layer unit, a green-sensitive layer unit, and blue-sensitive layer unit. However, the order of the arrangement may be reversed or an arrangement order in which color-sensitive layers having the same color sensitivity sandwich a light-sensitive layer of different color sensitivity, depending on purposes. A non-light-sensitive layer may be provided as an upper most layer, or lower most layer, and between the silver halide light-sensitive layers. These layers may contain a coupler, DIR compound, color-mixing inhibitor and etc, to be described later. In the plurality of silver halide emulsion layers constituting each unit light-sensitive layer, it is preferred that two layers consisting of a high-speed emulsion layer and a low-speed emulsion layer be arranged so that the speed is sequentially decreased toward a support as described in DE 1,121,470 or GB 923,045. Also, as described in JP-A's-57-112751, 62-200350, 62-206541 and 62-206543, layers can be arranged so that a low-speed emulsion layer is formed on a side remote from a support while a high-speed emulsion layer is formed on a side close to the support.

Specifically, layers can be arranged, from the farthest side from a support, in the order of low-speed blue-sensitive layer (BL)/high-speed blue-sensitive layer (BH)/high-speed

green-sensitive layer (GH)/low-speed green-sensitive layer (GL)/high-speed red-sensitive layer (RH)/low-speed red-sensitive layer (RL), or the order of BH/BL/GL/GH/RH/RL, or the order of BH/BL/GH/GL/RL/RH, or the like.

5 In addition, as described in JP-B-55-34932, layers can be arranged, from the farthest side from a support, in the order of blue-sensitive layer/GH/RH/GL/RL. Furthermore, as described in JP-A's-56-25738 and 62-63936, layers can be arranged, from the farthest side from a support, in the order of blue-sensitive layer/GL/RL/GH/RH.

10 As described in JP-B-49-15495, three layers can be arranged so that a silver halide emulsion layer having the highest speed is arranged as an upper layer, a silver halide emulsion layer having a speed lower than that of the upper layer is arranged as an inter layer, and a silver halide emulsion layer having a speed lower than that of the inter layer is arranged as a lower layer; i.e., three layers having different sensitivities can be arranged so that the speed is sequentially decreased toward the support. Even when a 15 layer structure is constituted by three layers having different sensitivities as mentioned above, these layers can be arranged in the order of medium-speed emulsion layer/high-speed emulsion layer/low-speed emulsion layer from the farthest side from a support in layers of the same color 20 sensitivity as described in JP-A-59-202464.

25 In addition, the layer arrangement can be made in the order of high-speed emulsion layer/low-speed emulsion layer/medium-speed emulsion layer, or in the order of low-speed emulsion layer/medium-speed emulsion layer/high-speed emulsion layer.

30 Furthermore, the layer arrangement can be changed as mentioned above even when four or more layers are formed.

35 It is preferable to utilize an inter layer inhibitory effect as means for improving a color reproduction.

40 It is also preferred to provide by coating a donor layer of the inter layer inhibitory effect to a red-sensitive layer. That is, it is preferred that  $\lambda_G$  of a green-sensitive silver halide emulsion layer, which is weight-average sensitivity wavelength of spectral sensitivity distribution of a green-sensitive silver halide emulsion layer, meets  $520 \text{ nm} < \lambda_G < 580 \text{ nm}$  and  $\lambda_{-R}$ , which is weight-average wavelength of spectral sensitivity distribution of an inter layer effect to a red-sensitive silver halide emulsion layer from other layers in a range of 45 500 nm to 600 nm, meets  $500 \text{ nm} < \lambda_{-R} < 560 \text{ nm}$ , and  $\lambda_G - \lambda_{-R}$  is 5 nm or more, preferably 10 nm or more.

$$50 \quad \lambda_G = \frac{\int_{500}^{600} \lambda S_G(\lambda) d\lambda}{\int_{500}^{600} S_G(\lambda) d\lambda}$$

55 In the formula,  $S_G(\lambda)$  signifies spectral sensitivity distribution curve of a green-sensitive silver halide emulsion layer.  $S_R$  at a specific wavelength  $\lambda$  is represented by an inverse number of an exposure amount that gives magenta density of fog+0.5 when the exposure was given at the specific wavelength.

60 In order to provide an inter layer effect to a red-sensitive layer at a specific wavelength range described above, it is preferable to separately provide an inter layer effect-donating layer containing silver halide grains that are spectrally sensitized with a given sensitivity. In order to realize the spectral sensitivity of the present invention, the weight-average sensitivity wavelength of the inter layer effect-donating layer is preferably set from 510 nm to 540 nm.

Herein, the weight-average wavelength  $\lambda_{\text{R}}$  of distribution of wavelength of the inter layer effect to a red-sensitive layer from other silver halide emulsion layers, may be determined by a method described in JP-B-3-10287.

In the present invention, the weight-average wavelength  $\lambda_{\text{R}}$  of a red-sensitive layer is preferably 630 nm or less. Herein, the weight-average wavelength  $\lambda_{\text{R}}$  of a red-sensitive layer is defined by the following formula (I):

$$\lambda_{\text{R}} = \frac{\int_{550}^{700} \lambda S_{\text{R}}(\lambda) d\lambda}{\int_{550}^{700} S_{\text{R}}(\lambda) d\lambda} \quad (\text{I})$$

In the formula,  $S_{\text{R}}(\lambda)$  signifies spectral sensitivity distribution curve of a red-sensitive silver halide emulsion layer, and  $S_{\text{R}}$  at a specific wavelength  $\lambda$  is represented by an inverse number of an exposure amount that gives cyan density of fog +0.5 when the exposure was given with the specific wavelength.

As a material for providing the inter layer effect, a compound that releases a development inhibitor or a precursor thereof through a reaction with an oxidized product of a developing agent obtained by development. For example, DIR (development inhibitor-releasing type) couplers, DIR-hydroquinones, couplers that release DIR-hydroquinone or precursor thereof may be used. When the development inhibitor has a high diffusibility, the development inhibiting effect may be attained wherever the donating layer is provided among a laminated multi-layer structure. However, a development inhibiting effect toward an unintended direction also arises. In order to compensate this, the donor layer is preferably a color-forming layer (e.g., a layer that forms the same color as the layer that suffers an undesired effect of the development inhibitor). In order to attain desired spectral sensitivity of the photosensitive material of the present invention, the inter layer effect-donating layer preferably forms magenta color.

The silver halide grains used in the inter layer effect-donating layer to red-sensitive layer are not particularly limited regarding, for example, the size thereof, and a shape, but so called tabular grains of a high aspect ratio or a monodisperse emulsion having a uniform grain size or silver iodobromide grains having a layer structure of iodide, are preferably used. Also, in order to enlarge exposure latitude, it is preferable to mix two or more kinds of emulsions having different grain sizes.

Although an inter layer effect-donating layer to a red-sensitive layer may be provided by coating on any position on a support, it is preferred that the interlayer-donating layer be provided by coating at a position which is closer to the support than the blue-sensitive layer and which is more remote from the support than the red-sensitive layer. It is further preferred that the interlayer-donating layer be positioned closer to the support than the yellow filter layer.

It is more preferred that the interlayer effect-donating layer to a red-sensitive layer be provided at a position which is closer to the support than the green-sensitive layer and which is more remote from the support than the red-sensitive layer. The interlayer-donating layer is most preferably arranged at a position adjacent to a side of the green-sensitive layer close to the support. The terminology "adjacent" used herein means that an inter layer or the like is not interposed therebetween.

There may be a plurality of interlayer effect-donating layers to a red-sensitive layer. These layers may be positioned so that they are adjacent to each other or are apart from each other.

5 In the present invention, use can be made of solid disperse dyes described in JP-A-11-305396.

The emulsions for use in the photosensitive material of the present invention may be any of the surface latent image type in which latent images are mainly formed in the 10 surface, the internal latent image type in which latent images are formed in the internal portion of grains and the type in which latent images exist in both the surface and the internal portion of grains. However, it is requisite that the emulsion be a negative type. The emulsion of the internal latent image 15 type may specifically be, for example, a core/shell internal-latent-image type emulsion described in JP-A-63-264740, whose preparation method is described in JP-A-59-133542. The thickness of the shell of this emulsion, although varied depending on development processing, etc., is preferably in 20 the range of 3 to 40 nm, more preferably 5 to 20 nm.

The silver halide emulsions are generally subjected to physical ripening, chemical sensitization and spectral sensitization before use. Additives employed in these steps are described in RD Nos. 17643, 18716 and 307105. Positions 25 where the description is made are listed in the following table.

In the photosensitive material of the present invention, two or more emulsions which are different from each other in at least one of the characteristics, specifically the grain 30 size, grain size distribution, halogen composition, grain configuration and speed of light-sensitive silver halide emulsion, can be mixed together and used in the same layer.

It is preferred that silver halide grains having a grain surface fogged as described in U.S. Pat. No. 4,082,553 and 35 silver halide grains or colloidal silver having a grain internal portion fogged as described in U.S. Pat. No. 4,626,498 and JP-A-59-214852 be used in light-sensitive silver halide emulsion layers and/or substantially non-light-sensitive hydrophilic colloid layers. The expression "silver halide 40 grains having a grain surface or grain internal portion fogged" refers to silver halide grains which can be developed uniformly (nonimagingewise) irrespective of the nonexposed or exposed zone of photosensitive material. The process for producing them is described in U.S. Pat. No. 4,626,498 and JP-A-59-214852. The silver halides constituting internal nuclei of core/shell silver halide grains having a grain internal portion fogged may have different halogen composition. Any of silver chloride, silver chlorobromide, silver iodobromide and silver chloroiodobromide can be 45 used as the silver halide having a grain surface or grain internal portion fogged. The average grain size of these fogged silver halide grains is preferably in the range of 0.01 to 0.75  $\mu\text{m}$ , more preferably 0.05 to 0.6  $\mu\text{m}$ . With respect to the grain configuration, although both regular grains and a 50 polydisperse emulsion can be used, monodispersity (at least 95% of the weight or number of silver halide grains have grain diameters falling within  $\pm 40\%$  of the average grain diameter) is preferred.

In the present invention, it is preferred to use non-light- 55 sensitive fine-grain silver halides. The expression "non-light-sensitive fine-grain silver halides" refers to silver halide fine grains which are not sensitive to light at the time of imagingewise exposure for obtaining dye images and which are substantially not developed at the time of development processing thereof. Those not having been fogged in advance are preferred. The fine-grain silver halides have a silver bromide content of 0 to 100 mol %, and, if necessary,

may contain silver chloride and/or silver iodide. Preferably, silver iodide is contained in an amount of 0.5 to 10 mol %. The average grain diameter (average of equivalent circular diameters of projected areas) of fine-grain silver halides is preferably in the range of 0.01 to 0.5  $\mu\text{m}$ , more preferably 0.02 to 0.2  $\mu\text{m}$ .

The fine-grain silver halides can be prepared by the same process as used in the preparation of common light-sensitive silver halides. It is not needed to optically sensitize the surface of silver halide grains. Further, any spectral sensitization thereof is also not needed. However, it is preferred to add known stabilizers, such as triazole-type, azaindene-type, benzothiazolium-type and mercapto-type compounds or zinc compounds, thereto prior to the addition of fine-grain silver halides to a coating liquid. Colloidal silver can be incorporated in layers containing fine-grain silver halides.

Various additives mentioned above are used in the photosensitive material regarding the technique of the invention, and other various additives may be used depending on purposes.

The additives are described in detail in Research Disclosure Item 17643 (December 1978), Item 18716 (November 1979) and Item 308119 (December 1989). A summary of the locations where they are described will be listed in the following table.

| Types of additives                                      | RD17643                  | RD18716                                                   | RD308119                                                    |
|---------------------------------------------------------|--------------------------|-----------------------------------------------------------|-------------------------------------------------------------|
| 1 Chemical sensitizing dyes                             | page 23                  | page 648<br>right column                                  | page 996                                                    |
| 2 Sensitivity-increasing agents                         |                          | page 648<br>right column                                  |                                                             |
| 3 Spectral sensitizing dye, super-sensitizers           | pages 23–24              | page 648,<br>right column<br>to page 649,<br>right column | page 996,<br>right column<br>to page 998,<br>right column   |
| 4 Brighteners                                           | page 24                  |                                                           | page 998<br>right column                                    |
| 5 Antifoggants, stabilizers                             | pages 24–25              | page 649<br>right column                                  | page 998,<br>right column<br>to page 1000,<br>right column  |
| 6 Light absorbents, filter dyes, ultraviolet absorbents | pages 25–26              | page 649,<br>right column<br>to page 650,<br>left column  | page 1003,<br>left column<br>to page 1003,<br>right column  |
| 7 Stain preventing agents                               | page 25,<br>right column | page 650,<br>left to<br>right columns                     | page 1002,<br>right column                                  |
| 8 Dye image stabilizers                                 | page 25                  |                                                           | page 1002,<br>right column                                  |
| 9 Film hardeners                                        | page 26                  | page 651,<br>left column                                  | page 1004,<br>right column<br>page 1005,<br>left column     |
| 10 Binders                                              | page 26                  | page 651,<br>left column                                  | page 1003,<br>right column<br>to page 1004,<br>right column |
| 11 Plasticizers, lubricants                             | page 27                  | page 650,<br>right column                                 | page 1006,<br>left to right<br>columns                      |
| 12 Coating aids, surfactants                            | pages 26–27              | page 650,<br>right column                                 | page 1005,<br>left column<br>to page 1006,<br>left column   |
| 13 Antistatic agents                                    | page 27                  | page 650,<br>right column                                 | page 1006,<br>right column<br>to page 1007,<br>left column  |

-continued

| Types of additives | RD17643 | RD18716 | RD308119                                                  |
|--------------------|---------|---------|-----------------------------------------------------------|
| 14 Matting agents  |         |         | page 1008,<br>left column<br>to page 1009,<br>left column |

- 10 With respect to the photosensitive material of the present invention and the emulsion suitable for use in the photosensitive material and also with respect to layer arrangement and related techniques, silver halide emulsions, dye forming couplers, DIR couplers and other functional couplers, various additives and development processing which can be used in the photographic photosensitive material, reference can be made to EP 0565096A1 (published on Oct. 13, 1993) and patents cited therein. Individual particulars and the locations where they are described will be listed below.
- 15 1. Layer arrangement: page 61 lines 23 to 35, page 61 line 41 to page 62 line 14,
- 20 2. Interlayers: page 61 lines 36 to 40,
- 25 3. Interlayer effect-donating layers: page 62 lines 15 to 18,
- 30 4. Silver halide halogen compositions: page 62 lines 21 to 25,
- 35 5. Silver halide grain crystal habits: page 62 lines 26 to 30,
- 40 6. Silver halide grain sizes: page 62 lines 31 to 34,
- 45 7. Emulsion preparation methods: page 62 lines 35 to 40,
- 50 8. Silver halide grain size distributions: page 62 lines 41 to 42,
- 55 9. Tabular grains: page 62 lines 43 to 46,
- 60 10. Internal structures of grains: page 62 lines 47 to 53,
- 65 11. Latent image forming types of emulsions: page 62 line 54 to page 63 to line 5,
- 70 12. Physical ripening and chemical sensitization of emulsion: page 63 lines 6 to 9,
- 75 13. Emulsion mixing: page 63 lines 10 to 13,
- 80 14. Fogged emulsions: page 63 lines 14 to 31,
- 85 15. Non light-sensitive emulsions: page 63 lines 32 to 43,
- 90 16. Silver coating amounts: page 63 lines 49 to 50,
- 95 17. Formaldehyde scavengers: page 64 lines 54 to 57,
- 100 18. Mercapto antifoggants: page 65 lines 1 to 2,
- 105 19. Fogging agent, etc. releasing agents: page 65 lines 3 to 7,
- 110 20. Dyes: page 65, lines 7 to 10,
- 115 21. Color coupler summary: page 65 lines 11 to 13,
- 120 22. Yellow, magenta and cyan couplers: page 65 lines 14 to 25,
- 125 23. Polymer couplers: page 65 lines 26 to 28,
- 130 24. Diffusive dye forming couplers: page 65 lines 29 to 31,
- 135 25. Colored couplers: page 65 lines 32 to 38,
- 140 26. Functional coupler summary: page 65 lines 39 to 44,
- 145 27. Bleaching accelerator-releasing couplers: page 65 lines 45 to 48,
- 150 28. Development accelerator-releasing couplers: page 65 lines 49 to 53,
- 155 29. Other DIR couplers: page 65 line 54 to page 66 to line 4,
- 160 30. Method of dispersing couplers: page 66 lines 5 to 28,
- 165 31. Antiseptic and mildewproofing agents: page 66 lines 29 to 33,
- 170 32. Types of photosensitive materials: page 66 lines 34 to 36,
- 175 33. Thickness of light-sensitive layer and swelling speed: page 66 line 40 to page 67 line 1,
- 180 34. Back layers: page 67 lines 3 to 8,
- 185 35. Development processing summary: page 67 lines 9 to 11,

36. Developing solutions and developing agents: page 67 lines 12 to 30,  
 37. Developing solution additives: page 67 lines 31 to 44,  
 38. Reversal processing: page 67 lines 45 to 56,  
 39. Processing solution open ratio: page 67 line 57 to page 68 line 12,  
 40. Development time: page 68 lines 13 to 15,  
 41. Bleach-fix, bleaching and fixing: page 68 line 16 to page 69 line 31,  
 42. Automatic processor: page 69 lines 32 to 40,  
 43. Washing, rinse and stabilization: page 69 line 41 to page 70 line 18,  
 44. Processing solution replenishment and reuse: page 70 lines 19 to 23,  
 45. Developing agent built-in sensitive material: page 70 lines 24 to 33,  
 46. Development processing temperature: page 70 lines 34 to 38, and  
 47. Application to film with lens: page 70 lines 39 to 41.

Moreover, preferred use can be made of a bleaching solution containing 2-pyridinecarboxylic acid or 2,6-pyridinedicarboxylic acid, a ferric salt such as ferric nitrate and a persulfate as described in EP 602,600. When this bleaching solution is used, it is preferred that the steps of stop and water washing be conducted between the steps of color development and bleaching. An organic acid such as acetic acid, succinic acid or maleic acid is preferably used as a stop solution. For pH adjustment and bleaching fog, it is preferred that the bleaching solution contains an organic acid such as acetic acid, succinic acid, maleic acid, glutaric acid or adipic acid in an amount of 0.1 to 2 mol/liter (hereinafter liter is referred to as "L", and milliliter is referred to as "mL").

A magnetic recording layer usable in the present invention will be described below.

This magnetic recording layer is formed by coating the surface of a support with an aqueous or organic solvent-based coating solution which is prepared by dispersing magnetic grains in a binder.

As the magnetic grains, it is possible to use grains of, e.g., ferromagnetic iron oxide such as  $\gamma\text{Fe}_2\text{O}_3$ , Co-deposited  $\gamma\text{Fe}_2\text{O}_3$ , Co-deposited magnetite, Co-containing magnetite, ferromagnetic chromium dioxide, a ferromagnetic metal, ferromagnetic alloy, Ba ferrite of a hexagonal system, Sr ferrite, Pb ferrite, and Ca ferrite. Co-deposited ferromagnetic iron oxide such as Co-deposited  $\gamma\text{Fe}_2\text{O}_3$  is preferable. The grain can take the shape of any of, e.g., a needle, rice grain, sphere, cube, and plate. The specific area is preferably  $20\text{ m}^2/\text{g}$  or more, and more preferably  $30\text{ m}^2/\text{g}$  or more as  $S_{BET}$ .

The saturation magnetization (as) of the ferromagnetic substance is preferably  $3.0 \times 10^4$  to  $3.0 \times 10^5\text{ A/m}$ , and especially preferably  $4.0 \times 10^4$  to  $2.5 \times 10^5\text{ A/m}$ . A surface treatment can be performed for the ferromagnetic grains by using silica and/or alumina or an organic material. Also, the surface of the ferromagnetic grain can be treated with a silane coupling agent or a titanium coupling agent as described in JP-A-6-161032. A ferromagnetic grain whose surface is coated with an inorganic or organic substance described in JP-A-4-259911 or 5-81652 can also be used.

As a binder used together with the magnetic grains, it is possible to use a thermoplastic resin described in JP-A-4-219569, thermosetting resin, radiation-curing resin, reactive resin, acidic, alkaline, or biodegradable polymer, natural polymer (e.g., a cellulose derivative and sugar derivative), and their mixtures. The Tg of the resin is  $-40^\circ\text{C}$ . to  $300^\circ\text{C}$ ., and its weight average molecular weight is 2,000 to 1,000,

000. Examples are a vinyl-based copolymer, cellulose derivatives such as cellulosediacetate, cellulosetriacetate, celluloseacetatepropionate, celluloseacetatebutylate, and cellulosetripropionate, acrylic resin, and polyvinylacetal resin. Gelatin is also preferable. Cellulosedi(tri)acetate is particularly preferable. This binder can be hardened by the addition of an epoxy-, aziridine-, or isocyanate-based crosslinking agent. Examples of the isocyanate-based crosslinking agent are isocyanates such as tolylenediisocyanate, 4,4'-diphenylmethanediisocyanate, hexamethylenediisocyanate, and xylylenediisocyanate, reaction products of these isocyanates and polyalcohol (e.g., a reaction product of 3 mols of tolylenediisocyanate and 1 mol of trimethylolpropane), and polyisocyanate produced by condensation of any of these isocyanates. These examples are described in JP-A-6-59357.

As a method of dispersing the magnetic substance in the binder, as described in JP-A-6-35092, a kneader, pin type mill, and annular mill are preferably used singly or together. 20 Dispersants described in JP-A-5-088283 and other known dispersants can be used. The thickness of the magnetic recording layer is 0.1 to 10  $\mu\text{m}$ , preferably 0.2 to 5  $\mu\text{m}$ , and more preferably 0.3 to 3  $\mu\text{m}$ . The weight ratio of the magnetic grains to the binder is preferably 0.5:100 to 60:100, and more preferably 1:100 to 30:100. The coating amount of the magnetic grains is 0.005 to 3  $\text{g/m}^2$ , preferably 0.01 to 2  $\text{g/m}^2$ , and more preferably 0.02 to 0.5  $\text{g/m}^2$ . The transmitting yellow density of the magnetic recording layer is preferably 0.01 to 0.50, more preferably 0.03 to 0.20, and especially preferably 0.04 to 0.15. The magnetic recording layer can be formed in the whole area of, or into the shape of stripes on, the back surface of a photographic support by coating or printing. As a method of coating the magnetic recording layer, it is possible to use any of an air doctor, 30 blade, air knife, squeegee, impregnation, reverse roll, transfer roll, gravure, kiss, cast, spray, dip, bar, and extrusion. A coating solution described in JP-A-5-341436 is preferable.

The magnetic recording layer can be given a lubricating property improving function, curling adjusting function, 40 antistatic function, adhesion preventing function, and head polishing function. Alternatively, another functional layer can be formed and these functions can be given to that layer. A polishing agent in which at least one type of grains are aspherical inorganic grains having a Mohs hardness of 5 or 45 more is preferable. The composition of this aspherical inorganic grain is preferably an oxide such as aluminum oxide, chromium oxide, silicon dioxide, titanium dioxide, and silicon carbide, a carbide such as silicon carbide and titanium carbide, or a fine powder of diamond. The surfaces 50 of the grains constituting these polishing agents can be treated with a silane coupling agent or titanium coupling agent. These grains can be added to the magnetic recording layer or overcoated (as, e.g., a protective layer or lubricant layer) on the magnetic recording layer. A binder used 55 together with the grains can be any of those described above and is preferably the same binder as in the magnetic recording layer. Sensitive materials having the magnetic recording layer are described in U.S. Pat. Nos. 5,336,589, 5,250,404, 5,229,259, and 5,215,874, and EP 466,130.

60 A polyester support used in the present invention will be described below. Details of the polyester support and sensitive materials, processing, cartridges, and examples (to be described later) are described in Journal of Technical Disclosure No. 94-6023 (JIII; 1994, Mar. 15). Polyester used in the present invention is formed by using diol and aromatic dicarboxylic acid as essential components. Examples of the aromatic dicarboxylic acid are 2,6-, 1,5-, 1,4-, and 2,7-

naphthalenedicarboxylic acids, terephthalic acid, isophthalic acid, and phthalic acid. Examples of the diol are diethyleneglycol, triethyleneglycol, cyclohexanedimethanol, bisphenol A, and bisphenol. Examples of the polymer are homopolymers such as polyethyleneterephthalate, polyethylenenaphthalate, and polycyclohexanedimethanol-terephthalate. Polyester containing 50 to 100 mol % of 2,6-naphthalenedicarboxylic acid is particularly preferable. Polyethylene-2,6-naphthalate is especially preferable among other polymers. The weight-average molecular weight ranges between about 5,000 and 200,000. The Tg of the polyester of the present invention is 50° C. or higher, preferably 90° C. or higher.

To give the polyester support a resistance to curling, the polyester support is heat-treated at a temperature of 40° C. to less than Tg, more preferably Tg-20° C. to less than Tg. The heat treatment can be performed at a fixed temperature within this range or can be performed together with cooling. The heat treatment time is 0.1 to 1500 hrs, more preferably 0.5 to 200 hrs. The heat treatment can be performed for a roll-like support or while a support is conveyed in the form of a web. The surface shape can also be improved by roughening the surface (e.g., coating the surface with conductive inorganic fine grains such as  $\text{SnO}_2$  or  $\text{Sb}_2\text{O}_5$ ). It is desirable to knurl and slightly raise the end portion, thereby preventing the cut portion of the core from being photographed. These heat treatments can be performed in any stage after support film formation, after surface treatment, after back layer coating (e.g., an antistatic agent or lubricating agent), and after undercoating. A preferable timing is after the antistatic agent is coated.

An ultraviolet absorbent can be incorporated into this polyester. Also, to prevent light piping, dyes or pigments such as Diaresin manufactured by Mitsubishi Kasei Corp. or Kayaset manufactured by NIPPON KAYAKU CO. LTD. commercially available for polyester can be incorporated.

In the present invention, it is preferable to perform a surface treatment in order to adhere the support and the sensitive material constituting layers. Examples of the surface treatment are surface activation treatments such as a chemical treatment, mechanical treatment, corona discharge treatment, flame treatment, ultraviolet treatment, high-frequency treatment, glow discharge treatment, active plasma treatment, laser treatment, mixed acid treatment, and ozone oxidation treatment. Among other surface treatments, the ultraviolet radiation treatment, flame treatment, corona treatment, and glow treatment are preferable.

An undercoating layer can include a single layer or two or more layers. Examples of an undercoating layer binder are copolymers formed by using, as a starting material, a monomer selected from vinylchloride, vinylidenechloride, butadiene, methacrylic acid, acrylic acid, itaconic acid, and maleic anhydride. Other examples are polyethyleneimine, an epoxy resin, grafted gelatin, nitrocellulose, and gelatin. Resorcin and p-chlorophenol are examples of a compound which swells a support. Examples of a gelatin hardener added to the undercoating layer are chromium salt (e.g., chromium alum), aldehydes (e.g., formaldehyde and glutaraldehyde), isocyanates, an active halogen compound (e.g., 2,4-dichloro-6-hydroxy-s-triazine), epichlorohydrin resin, and active vinylsulfone compound.  $\text{SiO}_2$ ,  $\text{TiO}_2$ , inorganic fine grains, or polymethylmethacrylate copolymer fine grains (0.01 to 10  $\mu\text{m}$ ) can also be contained as a matting agent.

In the present invention, an antistatic agent is preferably used. Examples of this antistatic agent are carboxylic acid, carboxylate, a macromolecule containing sulfonate, cationic macromolecule, and ionic surfactant compound.

As the antistatic agent, it is especially preferable to use fine grains of at least one crystalline metal oxide selected from  $\text{ZnO}$ ,  $\text{TiO}_2$ ,  $\text{SnO}_2$ ,  $\text{Al}_2\text{O}_3$ ,  $\text{In}_2\text{O}_3$ ,  $\text{SiO}_2$ ,  $\text{MgO}$ ,  $\text{BaO}$ ,  $\text{MoO}_3$ , and  $\text{V}_2\text{O}_5$ , and having a volume resistivity of  $10^7$   $\Omega\cdot\text{cm}$  or less, more preferably  $10^5$   $\Omega\cdot\text{cm}$  or less and a grain size of 0.001 to 1.0  $\mu\text{m}$ , fine grains of composite oxides (e.g.,  $\text{Sb}$ ,  $\text{P}$ ,  $\text{B}$ ,  $\text{In}$ ,  $\text{S}$ ,  $\text{Si}$ , and  $\text{C}$ ) of these metal oxides, fine grains of sol metal oxides, or fine grains of composite oxides of these sol metal oxides.

The content in a sensitive material is preferably to 500  $\text{mg}/\text{m}^2$ , and especially preferably 10 to 350  $\text{mg}/\text{m}^2$ . The ratio of a conductive crystalline oxide or its composite oxide to the binder is preferably 1/300 to 100/1, and more preferably 1/100 to 100/5.

A sensitive material of the present invention preferably has a slip property. Slip agent-containing layers are preferably formed on the surfaces of both a sensitive layer and back layer. A preferable slip property is 0.01 to 0.25 as a coefficient of kinetic friction. This represents a value obtained when a stainless steel sphere 5 mm in diameter is conveyed at a speed of 60 cm/min (25° C., 60% RH). In this evaluation, a value of nearly the same level is obtained when the surface of a sensitive layer is used as a sample to be measured.

Examples of a slip agent usable in the present invention are polyorganocyclohexane, higher fatty acid amide, higher fatty acid metal salt, and ester of higher fatty acid and higher alcohol. As the polyorganocyclohexane, it is possible to use, e.g., polydimethylcyclohexane, polydiethylcyclohexane, polystyrylmethylcyclohexane, or polymethylphenylcyclohexane. A layer to which the slip agent is added is preferably the outermost emulsion layer or back layer. Polydimethylcyclohexane or ester having a long-chain alkyl group is particularly preferable.

A sensitive material of the present invention preferably contains a matting agent. This matting agent can be added to either the emulsion surface or back surface and is especially preferably added to the outermost emulsion layer. The matting agent can be either soluble or insoluble in processing solutions, and the use of both types of matting agents is preferable. Preferable examples are polymethylmethacrylate grains, poly(methylmethacrylate/methacrylic acid)=9/1 or 5/5 (molar ratio) grains, and polystyrene grains. The grain size is preferably 0.8 to 10  $\mu\text{m}$ , and a narrow grain size distribution is preferable. It is preferable that 90% or more of all grains have grain sizes 0.9 to 1.1 times the average grain size. To increase the matting property, it is preferable to simultaneously add fine grains with a grain size of 0.8  $\mu\text{m}$  or smaller. Examples are polymethylmethacrylate grains (0.2  $\mu\text{m}$ ), poly(methylmethacrylate/methacrylic acid)=9/1 (molar ratio, 0.3  $\mu\text{m}$ ) grains, polystyrene grains (0.25  $\mu\text{m}$ ), and colloidal silica grains (0.03  $\mu\text{m}$ ).

The support used in the Examples may be prepared according to the method described in Example 1 of JP-2000-281815.

The film patrone employed in the present invention will be described below. The main material composing the patrone for use in the present invention may be a metal or a synthetic plastic.

Examples of preferable plastic materials include polystyrene, polyethylene, polypropylene and polyphenyl ether. The patrone for use in the present invention may contain various types of antistatic agents and can preferably contain, for example, carbon black, metal oxide grains, nonionic, anionic, cationic or betaine type surfactants and polymers. Such an antistatic patrone is described in JP-A's-1-312537 and 1-312538. The resistance thereof at 25° C. in 25% RH is preferably  $10^{12}$  Ω or less. The plastic patrone is generally molded from a plastic having carbon black or a pigment milled thereinto for imparting light shielding properties. The patrone size may be the same as the current size 135, or for miniaturization of cameras, it is advantageous to decrease the diameter of the 25 mm cartridge of the current size 135 to 22 mm or less. The volume of the case of the patrone is preferably 30 cm<sup>3</sup> or less, more preferably 25 cm<sup>3</sup> or less. The weight of the plastic used in each patrone or patrone case preferably ranges from 5 to 15 g.

The patrone for use in the present invention may be one capable of feeding a film out by rotating a spool. Further, the patrone may be so structured that a film front edge is accommodated in the main frame of the patrone and that the film front edge is fed from a port part of the patrone to the outside by rotating a spool shaft in a film feeding out direction. These are disclosed in U.S. Pat. Nos. 4,834,306 and 5,226,613. The photographic film for use in the present invention may be a generally so termed raw stock having not yet been developed or a developed photographic film. The raw stock and the developed photographic film may be accommodated in the same new patrone or in different patrones.

The color photographic lightsensitive material of the present invention is suitably used as a negative film for Advanced Photo System (hereinafter referred to as "AP system"). It is, for example, one obtained by working the film into AP system format and accommodating the same in a special purpose cartridge, such as NEXIA A, NEXIA F or NEXIA H (sequentially, ISO 200/100/400) produced by Fuji Photo Film Co., Ltd. (hereinafter referred to as "Fuji Film"). This cartridge film for AP system is charged in a camera for AP system such as Epion series, e.g., Epion 300Z, produced by Fuji Film and put to practical use. Moreover, the color photographic lightsensitive material of the present invention is suitable to a lens equipped film, such as Fuji Color Utsurundesu Super Slim (Quick Snap) produced by Fuji Film.

The thus photographed film is printed through the following steps in a minilabo system:

- (1) acceptance (receiving an exposed cartridge film from a customer),
- (2) detaching (transferring the film from the above cartridge to an intermediate cartridge for development),
- (3) film development,
- (4) re-attaching (returning the developed negative film to the original cartridge),
- (5) printing (continuous automatic printing of C/H/P three type print and index print on color paper (preferably, Super FA8 produced by Fuji Film)), and
- (6) collation and delivery (collating the cartridge and index print with ID number and delivering the same with prints).

The above system is preferably Fuji Film Minilabo Champion Super FA-298/FA-278/FA-258/FA-238 or Fuji Film Digital Labo System Frontier. Film processor of the Minilabo Champion is, for example, FP922AL/FP562B/FP562B, AL/FP362B/FP362B, AL, and recommended processing chemical is Fuji Color Just It CN-16L or CN-16Q. Printer processor is, for example, PP3008AR/PP3008A/PP1828AR/PP1828A/PP1258AR/PP1258A/PP72 8AR/PP728A, and recommended processing chemical thereof is Fuji Color Just It CP-47L or CP-40FAII.

In the Frontier System, use is made of scanner & image processor SP-1000 and laser printer & paper processor LP-1000P or Laser Printer LP-1000W. Fuji Film DT200/DT100 and AT200/AT100 are preferably used as detacher in the detaching step and as re-attacher in the reattaching step, respectively.

The AP system can be enjoyed by photo joy system whose center unit is Fuji Film digital image work station Aladdin 1000. For example, developed AP system cartridge film is directly charged in Aladdin 1000, or negative film, positive film or print image information is inputted with the use of 35 mm film scanner FE-550 or flat head scanner PE-550 therein, and obtained digital image data can easily be worked and edited. The resultant data can be outputted as prints by current labo equipment, for example, by means of digital color printer NC-550AL based on photofixing type thermal color printing system or Pictography 3000 based on laser exposure thermal development transfer system or through a film recorder. Moreover, Aladdin 1000 is capable of directly outputting digital information to a floppy disk or Zip disk or outputting it through a CD writer to CD-R.

On the other hand, at home, photographs can be enjoyed on TV only by charging the developed AP system cartridge film in photoplayer AP-1 manufactured by Fuji Film. Charging it in Photoscanner AS-1 manufactured by Fuji Film enables continuously feeding image information into a personal computer at a high speed. Further, Photovision FV-10/FV-5 manufactured by Fuji Film can be utilized for inputting a film, print or three-dimensional object in a personal computer. Still further, image information recorded on a floppy disk, Zip disk, CD-R or a hard disk can be enjoyed by conducting various workings on the personal computer by the use of Fuji Film Application Soft Photofactory. Digital color printer NC-2/NC-2D based on photofixing type thermal color printing system, manufactured by Fuji Film, is suitable for outputting high-quality prints from a personal computer.

Fuji Color Pocket Album AP-5 Pop L, AP-1 Pop L, AP-1 Pop KG or Cartridge File 16 is preferably employed for storing the developed AP system cartridge film.

Examples of the present invention will be described below, which, however, in no way limit the scope of the present invention.

#### EXAMPLE 1

Silver halide emulsions Em-A to Em-O specified in Table 1 were prepared with reference to the process for preparing emulsions Em-A to Em-O described in Example 1 of JP-A-2001-281815.

TABLE 1

| Emulsion name | Average AgI content (mol %) | Average equivalent sphere diameter ( $\mu\text{m}$ ) | Average aspect ratio | Average equivalent circle diameter ( $\mu\text{m}$ ) | Average grain thickness ( $\mu\text{m}$ ) | Shape   |
|---------------|-----------------------------|------------------------------------------------------|----------------------|------------------------------------------------------|-------------------------------------------|---------|
| A             | 4                           | 1.0                                                  | 25                   | 2.8                                                  | 0.11                                      | Tabular |
| B             | 5                           | 0.7                                                  | 15                   | 1.6                                                  | 0.11                                      | Tabular |
| C             | 4.7                         | 0.51                                                 | 7                    | 0.85                                                 | 0.12                                      | Tabular |
| D             | 1                           | 0.51                                                 | 11                   | 1.0                                                  | 0.09                                      | Tabular |
| E             | 5                           | 1.0                                                  | 25                   | 2.8                                                  | 0.11                                      | Tabular |
| F             | 5.5                         | 0.75                                                 | 15                   | 1.6                                                  | 0.11                                      | Tabular |
| G             | 4.7                         | 0.73                                                 | 9.9                  | 1.39                                                 | 0.14                                      | Tabular |
| H             | 2.5                         | 0.51                                                 | 9                    | 0.42                                                 | 0.10                                      | Tabular |
| I             | 1.5                         | 0.37                                                 | 9                    | 0.67                                                 | 0.074                                     | Tabular |
| J             | 5                           | 0.8                                                  | 12                   | 1.6                                                  | 0.13                                      | Tabular |
| K             | 3.7                         | 0.47                                                 | 3                    | 0.53                                                 | 0.18                                      | Tabular |
| L             | 5.5                         | 1.6                                                  | 12                   | 3.2                                                  | 0.27                                      | Tabular |
| M             | 8.8                         | 0.64                                                 | 5.2                  | 0.85                                                 | 0.16                                      | Tabular |
| N             | 3.7                         | 0.37                                                 | 4.6                  | 0.55                                                 | 0.12                                      | Tabular |
| O             | 1.8                         | 0.19                                                 | —                    | —                                                    | —                                         | Cubic   |

Referring to Table 1, dislocation lines as described in JP-A-3-237450 were observed in the tabular grains when the observation was conducted through a high-voltage electron microscope.

Emulsions Em-A1 and Em-A2 were prepared in the same manner as in the preparation of emulsion Em-A except that after the completion of chemical sensitization of emulsion Em-A, the temperature of the chemically sensitized emulsion was lowered to 40° C. and then electron-releasing compounds according to the present invention were added in the contents based on the quantity of silver contained in the emulsion, as specified in Table 2.

Similarly, emulsions Em-B1, B2, C1, C2, D1, D2, E1, E2, F1, F2, G1, G2, H1, H2, L1, L2, M1, M2, N1, N2, O1 and O2 were prepared except that after the completion of chemical sensitization of emulsions Em-B to H and Em-L to O, the temperature of the chemically sensitized emulsion was lowered to 40° C. and then electron-releasing compounds according to the present invention were added in the contents based on the quantity of silver contained in the emulsion, as specified in Table 2.

TABLE 2

| Emulsion number | Electron-releasing compound | Addition amount to silver amount (mol/mol-Ag) |
|-----------------|-----------------------------|-----------------------------------------------|
| Em-A1           | Exemplified compound 14     | $1 \times 10^{-6}$                            |
| Em-A2           | Exemplified compound 45     | $2 \times 10^{-6}$                            |
| Em-B1           | Exemplified compound 14     | $3 \times 10^{-6}$                            |
| Em-B2           | Exemplified compound 45     | $1 \times 10^{-6}$                            |
| Em-C1           | Exemplified compound 14     | $1 \times 10^{-6}$                            |
| Em-C2           | Exemplified compound 45     | $2 \times 10^{-6}$                            |
| Em-D1           | Exemplified compound 14     | $3 \times 10^{-6}$                            |
| Em-D2           | Exemplified compound 45     | $6 \times 10^{-6}$                            |
| Em-E1           | Exemplified compound 14     | $1 \times 10^{-6}$                            |
| Em-E2           | Exemplified compound 45     | $2 \times 10^{-6}$                            |
| Em-F1           | Exemplified compound 14     | $4 \times 10^{-6}$                            |
| Em-F2           | Exemplified compound 45     | $4 \times 10^{-6}$                            |
| Em-G1           | Exemplified compound 14     | $5 \times 10^{-6}$                            |
| Em-G2           | Exemplified compound 45     | $7 \times 10^{-6}$                            |
| Em-H1           | Exemplified compound 14     | $3 \times 10^{-6}$                            |
| Em-H2           | Exemplified compound 45     | $8 \times 10^{-6}$                            |
| Em-L1           | Exemplified compound 7      | $4 \times 10^{-6}$                            |
| Em-L2           | Exemplified compound 37     | $5 \times 10^{-6}$                            |
| Em-M1           | Exemplified compound 7      | $6 \times 10^{-6}$                            |
| Em-M2           | Exemplified compound 37     | $4 \times 10^{-6}$                            |
| Em-N1           | Exemplified compound 7      | $7 \times 10^{-6}$                            |

TABLE 2-continued

| Emulsion number | Electron-releasing compound | Addition amount to silver amount (mol/mol-Ag) |
|-----------------|-----------------------------|-----------------------------------------------|
| Em-N2           | Exemplified compound 37     | $9 \times 10^{-6}$                            |
| Em-O1           | Exemplified compound 7      | $5 \times 10^{-6}$                            |
| Em-O2           | Exemplified compound 37     | $4 \times 10^{-6}$                            |

## (Preparation of Sample 101)

A triacetylcellulose support was coated with multiple layers of the following respective compositions, thereby obtaining a color negative film (sample 101).

## (Composition of Light-Sensitive Layer)

Main materials used in each of the layers are classified as follows:

ExC: cyan coupler, UV: ultraviolet absorber,  
ExM: magenta coupler, HBS: high b.p. org. solvent,  
ExY: yellow coupler, H: gelatin hardener.

(For each specific compound, in the following description, figure is assigned after the character, and the chemical formula thereof is shown thereafter).

The numeric value given beside the description of each component is for the coating amount expressed in the unit of  $\text{g}/\text{m}^2$ . With respect to the silver halides, the coating amount is in terms of silver quantity.

| 1st layer (First antihalation layer)                                                                      |        |       |    |
|-----------------------------------------------------------------------------------------------------------|--------|-------|----|
| Black colloidal silver                                                                                    | silver | 0.127 | 55 |
| Silver iodobromide emulsion (av. equiv. sphere diam: 0.07 $\mu\text{m}$ , silver iodide content: 2 mol %) | silver | 0.008 |    |
| Gelatin                                                                                                   |        | 0.900 |    |
| ExC-1                                                                                                     |        | 0.002 |    |
| ExC-3                                                                                                     |        | 0.002 |    |
| Cpd-2                                                                                                     |        | 0.001 |    |
| HBS-1                                                                                                     |        | 0.005 | 60 |
| HBS-2                                                                                                     |        | 0.002 |    |
| F-8                                                                                                       |        | 0.001 |    |
| 2nd layer (Second antihalation layer)                                                                     |        |       |    |
| Black colloidal silver                                                                                    | silver | 0.019 | 65 |
| Gelatin                                                                                                   |        | 0.425 |    |
| ExF-1                                                                                                     |        | 0.002 |    |

-continued

|                                                                                       |        |       |    |  |
|---------------------------------------------------------------------------------------|--------|-------|----|--|
| Solid disperse dye ExF-9                                                              |        | 0.120 |    |  |
| HBS-1                                                                                 |        | 0.074 |    |  |
| F-8                                                                                   |        | 0.001 |    |  |
| <u>3rd layer (Interlayer)</u>                                                         |        |       | 5  |  |
| Cpd-1                                                                                 |        | 0.080 |    |  |
| HBS-1                                                                                 |        | 0.042 |    |  |
| Gelatin                                                                               |        | 0.300 |    |  |
| <u>4th layer (Low-speed red-sensitive emulsion layer)</u>                             |        |       | 10 |  |
| Em-D                                                                                  | silver | 0.407 |    |  |
| Em-C                                                                                  | silver | 0.457 |    |  |
| ExC-1                                                                                 |        | 0.233 |    |  |
| ExC-2                                                                                 |        | 0.026 |    |  |
| ExC-3                                                                                 |        | 0.129 |    |  |
| ExC-4                                                                                 |        | 0.155 |    |  |
| ExC-5                                                                                 |        | 0.029 |    |  |
| ExC-6                                                                                 |        | 0.013 |    |  |
| Cpd-2                                                                                 |        | 0.025 |    |  |
| Cpd-4                                                                                 |        | 0.025 |    |  |
| ExC-8                                                                                 |        | 0.050 |    |  |
| HBS-1                                                                                 |        | 0.114 |    |  |
| HBS-5                                                                                 |        | 0.038 |    |  |
| Gelatin                                                                               |        | 1.474 |    |  |
| <u>5th layer (Medium-speed red-sensitive emulsion layer)</u>                          |        |       |    |  |
| Em-B                                                                                  | silver | 0.601 |    |  |
| Em-C                                                                                  | silver | 0.301 |    |  |
| ExC-1                                                                                 |        | 0.154 |    |  |
| ExC-2                                                                                 |        | 0.037 |    |  |
| ExC-3                                                                                 |        | 0.018 |    |  |
| ExC-4                                                                                 |        | 0.103 |    |  |
| ExC-5                                                                                 |        | 0.037 |    |  |
| ExC-6                                                                                 |        | 0.050 |    |  |
| Cpd-2                                                                                 |        | 0.036 |    |  |
| Cpd-4                                                                                 |        | 0.028 |    |  |
| Cpd-6                                                                                 |        | 0.060 |    |  |
| ExC-7                                                                                 |        | 0.010 |    |  |
| HBS-1                                                                                 |        | 0.129 |    |  |
| Gelatin                                                                               |        | 1.086 |    |  |
| <u>6th layer (High-speed red-sensitive emulsion layer)</u>                            |        |       | 35 |  |
| Em-A                                                                                  | silver | 0.950 |    |  |
| ExC-1                                                                                 |        | 0.072 |    |  |
| ExC-3                                                                                 |        | 0.035 |    |  |
| ExC-10                                                                                |        | 0.080 |    |  |
| Cpd-2                                                                                 |        | 0.064 |    |  |
| Cpd-4                                                                                 |        | 0.077 |    |  |
| Cpd-6                                                                                 |        | 0.060 |    |  |
| ExC-7                                                                                 |        | 0.040 |    |  |
| HBS-1                                                                                 |        | 0.329 |    |  |
| HBS-2                                                                                 |        | 0.120 |    |  |
| Gelatin                                                                               |        | 1.245 |    |  |
| <u>7th layer (Interlayer)</u>                                                         |        |       |    |  |
| Cpd-1                                                                                 |        | 0.094 |    |  |
| Cpd-7                                                                                 |        | 0.369 |    |  |
| A-1                                                                                   |        | 0.043 |    |  |
| Solid disperse dye ExF-4                                                              |        | 0.030 |    |  |
| HBS-1                                                                                 |        | 0.049 |    |  |
| Polyethyl acrylate latex                                                              |        | 0.088 |    |  |
| Gelatin                                                                               |        | 0.886 |    |  |
| <u>8th layer (Layer capable of exerting interlayer effect on red-sensitive layer)</u> |        |       | 55 |  |
| Em-J                                                                                  | silver | 0.300 |    |  |
| Em-K                                                                                  | silver | 0.200 |    |  |
| Cpd-4                                                                                 |        | 0.030 |    |  |
| ExM-2                                                                                 |        | 0.057 |    |  |
| ExM-3                                                                                 |        | 0.016 |    |  |
| ExM-4                                                                                 |        | 0.051 |    |  |
| ExY-1                                                                                 |        | 0.008 |    |  |
| ExY-6                                                                                 |        | 0.042 |    |  |
| ExC-9                                                                                 |        | 0.011 |    |  |
| HBS-1                                                                                 |        | 0.090 |    |  |
| HBS-3                                                                                 |        | 0.003 |    |  |
| HBS-5                                                                                 |        | 0.030 |    |  |
| Gelatin                                                                               |        | 0.610 |    |  |

-continued

|  |  |  |    |                                                                 |        |       |
|--|--|--|----|-----------------------------------------------------------------|--------|-------|
|  |  |  |    | <u>9th layer (Low-speed green-sensitive emulsion layer)</u>     |        |       |
|  |  |  | 5  | Em-H                                                            | silver | 0.200 |
|  |  |  |    | Em-G                                                            | silver | 0.220 |
|  |  |  |    | Em-I                                                            | silver | 0.130 |
|  |  |  |    | ExM-2                                                           |        | 0.378 |
|  |  |  |    | ExM-3                                                           |        | 0.047 |
|  |  |  |    | ExY-1                                                           |        | 0.009 |
|  |  |  | 10 | ExC-9                                                           |        | 0.007 |
|  |  |  |    | HBS-1                                                           |        | 0.098 |
|  |  |  |    | HBS-3                                                           |        | 0.010 |
|  |  |  |    | HBS-4                                                           |        | 0.077 |
|  |  |  |    | HBS-5                                                           |        | 0.548 |
|  |  |  |    | Cpd-5                                                           |        | 0.010 |
|  |  |  |    | Gelatin                                                         |        | 1.470 |
|  |  |  |    | <u>10th layer (Medium-speed green-sensitive emulsion layer)</u> |        |       |
|  |  |  | 15 | Em-F                                                            | silver | 0.536 |
|  |  |  |    | ExM-2                                                           |        | 0.049 |
|  |  |  |    | ExM-3                                                           |        | 0.035 |
|  |  |  |    | ExM-4                                                           |        | 0.014 |
|  |  |  | 20 | ExY-1                                                           |        | 0.003 |
|  |  |  |    | ExY-5                                                           |        | 0.006 |
|  |  |  |    | ExC-6                                                           |        | 0.007 |
|  |  |  |    | ExC-8                                                           |        | 0.010 |
|  |  |  |    | ExC-9                                                           |        | 0.012 |
|  |  |  |    | HBS-1                                                           |        | 0.065 |
|  |  |  | 25 | HBS-3                                                           |        | 0.002 |
|  |  |  |    | HBS-5                                                           |        | 0.020 |
|  |  |  |    | Cpd-5                                                           |        | 0.004 |
|  |  |  |    | Gelatin                                                         |        | 0.446 |
|  |  |  |    | <u>11th layer (High-speed green-sensitive emulsion layer)</u>   |        |       |
|  |  |  | 30 | Em-E                                                            | silver | 0.493 |
|  |  |  |    | Em-G                                                            | silver | 0.440 |
|  |  |  |    | ExC-7                                                           |        | 0.010 |
|  |  |  |    | ExM-1                                                           |        | 0.022 |
|  |  |  |    | ExM-2                                                           |        | 0.045 |
|  |  |  |    | ExM-3                                                           |        | 0.014 |
|  |  |  |    | ExM-4                                                           |        | 0.010 |
|  |  |  |    | ExM-5                                                           |        | 0.010 |
|  |  |  |    | Cpd-3                                                           |        | 0.004 |
|  |  |  |    | Cpd-4                                                           |        | 0.007 |
|  |  |  |    | Cpd-5                                                           |        | 0.010 |
|  |  |  |    | HBS-1                                                           |        | 0.148 |
|  |  |  | 40 | HBS-5                                                           |        | 0.037 |
|  |  |  |    | Polyethyl acrylate latex                                        |        | 0.099 |
|  |  |  |    | Gelatin                                                         |        | 0.939 |
|  |  |  |    | <u>12th layer (Yellow filter layer)</u>                         |        |       |
|  |  |  |    | Cpd-1                                                           |        | 0.094 |
|  |  |  |    | Solid disperse dye ExF-2                                        |        | 0.150 |
|  |  |  |    | Solid disperse dye ExF-5                                        |        | 0.010 |
|  |  |  |    | Oil soluble dye ExF-7                                           |        | 0.010 |
|  |  |  |    | HBS-1                                                           |        | 0.049 |
|  |  |  |    | A-1                                                             |        | 0.043 |
|  |  |  |    | Gelatin                                                         |        | 0.630 |
|  |  |  |    | <u>13th layer (Low-speed blue-sensitive emulsion layer)</u>     |        |       |
|  |  |  | 50 | Em-O                                                            | silver | 0.060 |
|  |  |  |    | Em-M                                                            | silver | 0.404 |
|  |  |  |    | Em-N                                                            | silver | 0.076 |
|  |  |  |    | ExC-1                                                           |        | 0.048 |
|  |  |  |    | ExY-1                                                           |        | 0.012 |
|  |  |  |    | ExY-2                                                           |        | 0.350 |
|  |  |  |    | ExY-6                                                           |        | 0.060 |
|  |  |  |    | ExY-7                                                           |        | 0.300 |
|  |  |  |    | ExC-9                                                           |        | 0.012 |
|  |  |  | 60 | Cpd-2                                                           |        | 0.100 |
|  |  |  |    | Cpd-3                                                           |        | 0.004 |
|  |  |  |    | HBS-1                                                           |        | 0.222 |
|  |  |  |    | HBS-5                                                           |        | 0.074 |
|  |  |  |    | Gelatin                                                         |        | 2.058 |
|  |  |  |    | <u>14th layer (High-speed blue-sensitive emulsion layer)</u>    |        |       |
|  |  |  | 65 | Em-L                                                            | silver | 0.974 |
|  |  |  |    | ExY-2                                                           |        | 0.100 |
|  |  |  |    | ExY-7                                                           |        | 0.100 |
|  |  |  |    | Cpd-2                                                           |        | 0.075 |

-continued

|                                                                                                           |        |                      |    |
|-----------------------------------------------------------------------------------------------------------|--------|----------------------|----|
| Cpd-3                                                                                                     |        | 0.001                |    |
| HBS-1                                                                                                     |        | 0.071                |    |
| Gelatin                                                                                                   |        | 0.678                |    |
| <u>15th layer (First protective layer)</u>                                                                |        |                      |    |
| Silver iodobromide emulsion (av. equiv. sphere diam: 0.07 $\mu\text{m}$ , silver iodide content: 2 mol %) | silver | 0.280                |    |
| UV-1                                                                                                      |        | 0.100                | 10 |
| UV-2                                                                                                      |        | 0.060                |    |
| UV-3                                                                                                      |        | 0.095                |    |
| UV-4                                                                                                      |        | 0.013                |    |
| UV-5                                                                                                      |        | 0.200                |    |
| F-11                                                                                                      |        | 0.009                |    |
| S-1                                                                                                       |        | 0.086                |    |
| HBS-1                                                                                                     |        | 0.175                |    |
| HBS-4                                                                                                     |        | 0.050                |    |
| Gelatin                                                                                                   |        | 1.984                |    |
| <u>16th layer (Second protective layer)</u>                                                               |        |                      |    |
| H-1                                                                                                       |        | 0.400                |    |
| B-1 (diameter 1.7 $\mu\text{m}$ )                                                                         |        | 0.050                |    |
| B-2 (diameter 1.7 $\mu\text{m}$ )                                                                         |        | 0.150                |    |
| B-3                                                                                                       |        | 0.050                |    |
| W-5                                                                                                       |        | 0.025                |    |
| W-1                                                                                                       |        | $9.0 \times 10^{-3}$ |    |
| S-1                                                                                                       |        | 0.200                |    |
| Gelatin                                                                                                   |        | 0.750                |    |

In addition, B-4 to B-6, F-1 to F-17, a lead salt, a platinum salt, an iridium salt and a rhodium salt were appropriately added to the individual layers in order to improve the storage life, processability, resistance to pressure, antiseptic and mildewproofing properties, antistatic properties and coating property thereof.

Preparation of dispersion of organic solid disperse dye:

The ExF-2 of the 12th layer was dispersed by the following method. Specifically,

|    |  |                                                                        |          |
|----|--|------------------------------------------------------------------------|----------|
| 5  |  |                                                                        |          |
|    |  | Wet cake of ExF-2 (containing 17.6 wt. % water)                        | 2.800 kg |
|    |  | Sodium octylphenyldiethoxymethanesulfonate (31 wt. % aqueous solution) | 0.376 kg |
| 10 |  | F-15 (7% aqueous solution)                                             | 0.011 kg |
|    |  | Water                                                                  | 4.020 kg |
|    |  | Total                                                                  | 7.210 kg |
| 15 |  | (adjusted to pH = 7.2 with NaOH).                                      |          |

Slurry of the above composition was agitated by means of a dissolver to thereby effect a preliminary dispersion, and further dispersed by means of agitator mill LMK-4 under such conditions that the peripheral speed, delivery rate and packing ratio of 0.3 mm-diameter zirconia beads were 10 m/s, 0.6 kg/min and 80%, respectively, until the absorbance ratio of the dispersion became 0.29. Thus, a solid particulate dispersion was obtained, wherein the average particle diameter of dye particulate was 0.29  $\mu\text{m}$ .

Solid dispersions of ExF-4 and ExF-9 were obtained in the same manner. The average particle diameters of these dye particulates were 0.28  $\mu\text{m}$  and 0.49  $\mu\text{m}$ , respectively. ExF-5 was dispersed by the microprecipitation dispersion method described in Example 1 of EP. No. 549,489A. The average particle diameter thereof was 0.06  $\mu\text{m}$ .

Compounds used in the preparation of each layer are shown below.

ExC-1



ExC-2



-continued

ExC-3

ExC-4



ExC-5

ExC-6



ExC-7

ExC-8



ExC-9

ExC-10



ExM-1



-continued

ExM-2



ExM-3



ExM-4



ExM-5



-continued

ExY-1



ExY-2



ExY-5



ExY-6



-continued

ExY-7

Cpd-1



Cpd-2



Cpd-3



Cpd-4



Cpd-5



Cpd-6

UV-1



UV-2



UV-3



UV-4



UV-5



-continued

B-1

B-2



$x/y = 10/90$  (Wt. ratio)  
Weight-average mol. wt.:  
about 35,000



$x/y = 40/60$  (Wt. ratio)  
Weight-average mol. wt.:  
about 20,000

B-3

H-1



(Mol. ratio)  
Weight-average mol. wt.:  
about 8,000



S-1

HBS-1



Tricresyl phosphate

HBS-2

HBS-3

Di (n-butyl) phthalate



HBS-4

HBS-5

Tri (2-ethylhexyl) phosphate



F-1

F-2





-continued

W-5

B-4



Weight-average mol. wt.:  
about 750,000

B-5

B-6



$x/y = 70/30$  (Wt. ratio)  
Weight-average mol. wt.:  
about 17,000



Weight-average mol. wt.:  
about 10,000

Cpd-7

ExF-1



ExF-2

ExF-4



ExF-5

ExF-7



ExF-9



-continued

A-1



The thus prepared color negative photosensitive material 15 was referred to as sample 101.

(Preparation of Samples 102 to 115)

Samples 102 to 115 each having at a density of Dmin+0.5 a spectral sensitivity distribution of blue-sensitive layer as specified in Table 3 were prepared by effecting equal-silver-quantity changes of the emulsions Em-0, Em-M and Em-N of the 13th layer and the emulsion Em-L of the 14th layer to emulsions Em-O1, Em-M1, Em-N1 and Em-L1, respectively, or emulsions Em-O2, Em-M2, Em-N2 and Em-L2, respectively, and further by changing the amount of compounds UV-1 to -5 in the 15th layer (first protective layer) so as to change the spectral sensitivity in the ultraviolet region.

With respect to the thus obtained samples, the film speed, charge conditioning capability and radiation tolerance were estimated.

(Estimation of Speed)

Each of the samples was exposed through gelatin filter SC-39 (long-wavelength light transmission filter of 390 nm cutoff wavelength) produced by Fuji Photo Film Co., Ltd. and a continuous wedge for  $\frac{1}{100}$  sec. The exposed samples were developed with the use of automatic processor FP-360B manufactured by Fuji Photo Film Co., Ltd. under the following conditions.

With respect to the processed samples, the density thereof was measured through a blue filter to thereby estimate the photographic characteristics thereof.

The film speed was expressed by the relative value, in logarithmic number, of inverse number of exposure amount required for reaching a density of fog density plus 0.2 (the speed of sample 101 was assumed to be a control).

(Estimation of Charge Conditioning Capability)

Each of the samples was wrought into 135-format, placed in a film cartridge and charged in a camera. High-speed winding was performed in an atmosphere of 15° C. temperature and 15% humidity, and film development was carried out by the following processing. The developed samples were visually inspected with respect to fog.

(Estimation of Radiation Tolerance)

The coating samples 101 to 115 were exposed to 0.2 R  $\gamma$ -radiation (1.173, 1.333 MeV) from radioactive isotope element Co<sup>60</sup>. The exposed samples were developed by the same processing as mentioned above, and with respect to the developed samples, the value of fog density was determined by carrying out density measurement through a blue filter. The fog increase attributed to the exposure to radiation was calculated from this fog value and the fog density of samples used in the above film speed estimation. The radiation tolerance was estimated by the relative value of fog increase on the basis of that of the sample 101.

15 The processing steps and compositions of processing solutions are as follows.

(Processing Steps)

| Step              | Time            | Temp.    | Qty. Of replenisher* | Tank volume |
|-------------------|-----------------|----------|----------------------|-------------|
| Color             | 3 min           | 37.8° C. | 20 mL                | 11.5 L      |
| Development       | 5 sec           |          |                      |             |
| Bleaching         | 50 sec          | 38.0° C. | 5 mL                 | 5 L         |
| Fixing (1)        | 50 sec          | 38.0° C. | —                    | 5 L         |
| Fixing (2)        | 50 sec          | 38.0° C. | 8 mL                 | 5 L         |
| Washing           | 30 sec          | 38.0° C. | 17 mL                | 3 L         |
| Stabilization (1) | 20 sec          | 38.0° C. | —                    | 3 L         |
| Stabilization (2) | 20 sec          | 38.0° C. | 15 mL                | 3 L         |
| Drying            | 1 min<br>30 sec | 60° C.   |                      |             |

35 \*The replenishment rate is a value per 1.1 m of a 35-mm wide photosensitive material (equivalent to one role of 24 Ex. film).

The stabilizer was fed from stabilization (2) to stabilization (1) by counter current. All the overflow of washing water was introduced into fixing bath (2). The amounts of 40 drag-in of developer into the bleaching step, drag-in of of bleaching solution into the fixing step and drag-in of fixer into the washing step were 2.5 mL, 2.0 mL and 2.0 mL, respectively, per 1.1 m of a 35-mm wide photosensitive material. Each crossover time was 6 sec, which was included in the processing time of the previous step.

The open area of the above processor was 100 cm<sup>2</sup> for the color developer, 120 cm<sup>2</sup> for the bleaching solution and about 100 cm<sup>2</sup> for the other processing solutions.

45 The composition of each of the processing solutions was as follows.

|                                                  | Tank solution (g) | Replenisher(g) |
|--------------------------------------------------|-------------------|----------------|
| <u>(Color developer)</u>                         |                   |                |
| Diethylenetriamine-pentaacetic acid              | 3.0               | 3.0            |
| Disodium catechol-3,5-disulfonate                | 0.3               | 0.3            |
| Sodium sulfite                                   | 3.9               | 5.3            |
| Potassium carbonate                              | 39.0              | 39.0           |
| Disodium-N,N-bis (2-sulfonatoethyl)hydroxylamine | 1.5               | 2.0            |
| Potassium bromide                                | 1.3               | 0.3            |
| Potassium iodide                                 | 1.3 mg            | —              |
| 4-Hydroxy-6-methyl-1,3,3a,7-tetrazaindene        | 0.05              | —              |

-continued

|                                                                                           | Tank solution (g) | Replenisher(g) |
|-------------------------------------------------------------------------------------------|-------------------|----------------|
| Hydroxylamine sulfate                                                                     | 2.4               | 3.3            |
| 2-Methyl-4-[N-ethyl-N-( $\beta$ -hydroxyethyl)amino]-aniline sulfate                      | 4.5               | 6.5            |
| Water to make                                                                             | 1.0 L             | 1.0 L          |
| pH (adjusted by the use of potassium hydroxide and sulfuric acid)<br>(Bleaching solution) | 10.05             | 10.18          |
| Fe(III) ammonium 1,3-diamino-propanetetraacetate monohydrate                              | 113               | 170            |
| Ammonium bromide                                                                          | 70                | 105            |
| Ammonium nitrate                                                                          | 14                | 21             |
| Succinic acid                                                                             | 34                | 51             |
| Maleic acid                                                                               | 28                | 42             |
| Water to make                                                                             | 1.0 L             | 1.0 L          |
| pH (adjusted by the use of aqueous ammonia)<br>(Fixing (1) tank solution)                 | 4.6               | 4.0            |

5.95 (by volume) mixture of the above bleaching tank solution and the following fixing tank solution (pH 6.8)  
(Fixing (2))

|                                                    | Tank solution (g) | Replenisher(g) |
|----------------------------------------------------|-------------------|----------------|
| Aqueous solution of ammonium thiosulfate (750 g/L) | 240 mL            | 720 mL         |
| Imidazole                                          | 7                 | 21             |
| Ammonium methanethiosulfonate                      | 5                 | 15             |
| Ammonium methanesulfonate                          | 10                | 30             |
| Ethylenediaminetetraacetic acid                    | 13                | 39             |
| Water to make                                      | 1.0 L             | 1.0 L          |

-continued

|   | Tank solution (g)                                                              | Replenisher(g) |
|---|--------------------------------------------------------------------------------|----------------|
| 5 | pH (adjusted by the use of aqueous ammonia and acetic acid)<br>(Washing water) | 7.4            |

10 Tap water was passed through a mixed-bed column filled with H-type strongly acidic cation exchange resin (Amberlite IR-120B produced by Rohm & Haas Co.) and OH-type strongly basic anion exchange resin (Amberlite IR-400 produced by the same maker) so as to set the concentration of calcium and magnesium ions at 3 mg/L or less. Subsequently, 20 mg/L of sodium dichloroisocyanurate and 150 mg/L of sodium sulfate were added. The pH of the solution ranged from 6.5 to 7.5.

20

(Stabilizer): common to tank solution and replenisher

|    | (g)                                                                      |
|----|--------------------------------------------------------------------------|
| 25 | Sodium p-toluenesulfonate                                                |
|    | Polyoxyethylene p-mononylphenyl ether (average polymerization degree 10) |
|    | Sodium salt of 1,2-benzoisothiazolin-3-one                               |
|    | Disodium ethylenediaminetetraacetate                                     |
|    | 1,2,4-triazole                                                           |
| 30 | 1,4-bis(1,2,4-triazol-1-ylmethyl)-piperazine                             |
|    | Water to make                                                            |
|    | pH                                                                       |

TABLE 3

| Sample | Electron-releasing compound | $S_B(370 \text{ nm})/S_B(420 \text{ nm})$ | Relative speed | static-induced fog | Increment in fog due to radiation | Remarks |
|--------|-----------------------------|-------------------------------------------|----------------|--------------------|-----------------------------------|---------|
| 101    | None                        | 0.76                                      | 100            | X                  | 100                               | Comp.   |
| 102    | None                        | 0.65                                      | 99             | Δ                  | 98                                | Comp.   |
| 103    | None                        | 0.57                                      | 99             | Δ                  | 96                                | Comp.   |
| 104    | None                        | 0.44                                      | 101            | ○                  | 95                                | Comp.   |
| 105    | None                        | 0.22                                      | 100            | ○                  | 84                                | Comp.   |
| 106    | Exemplified compound 7      | 0.75                                      | 151            | XX                 | 120                               | Comp.   |
| 107    | Exemplified compound 7      | 0.65                                      | 152            | Δ                  | 110                               | Inv.    |
| 108    | Exemplified compound 7      | 0.57                                      | 155            | ○                  | 100                               | Inv.    |
| 109    | Exemplified compound 7      | 0.43                                      | 153            | ○                  | 91                                | Inv.    |
| 110    | Exemplified compound 7      | 0.22                                      | 150            | ○                  | 87                                | Inv.    |
| 111    | Exemplified compound 37     | 0.77                                      | 139            | XX                 | 131                               | Comp.   |
| 112    | Exemplified compound 37     | 0.65                                      | 140            | Δ                  | 119                               | Inv.    |
| 113    | Exemplified compound 37     | 0.57                                      | 140            | ○                  | 95                                | Inv.    |
| 114    | Exemplified compound 37     | 0.46                                      | 136            | ○                  | 91                                | Inv.    |
| 115    | Exemplified compound 37     | 0.21                                      | 139            | ○                  | 85                                | Inv.    |

○: No fog arose;  
○: Very slight fog arose;  
Δ: Slight fog arose;  
X: Much fog arose.

With respect to the samples 101 to 115, the results of relative sensitivity, charge conditioning capability characteristics and radiation tolerance are listed in Table 3.

As apparent from Table 3, in the Comparative Examples, the addition of electron-releasing compound, although exerting a high sensitivity increasing effect, intensifies the static-induced fog and radiation-induced fog. In the present invention, it is seen that the excellence in static tolerance and radiation tolerance while maintaining the advantage of sensitivity increase is realized through achieving of the spectral sensitivity distribution of the present invention by, while adding an electron-releasing compound, increasing the amount of ultraviolet absorber used.

## EXAMPLE 2

Samples 201 to 206 were prepared in the same manner as in the preparation of samples 110 and 115 except that the compound W-1 of the 16th layer (second protective layer) was replaced in equivalent weight by compounds specified in Table 4.

With respect to the samples 110, 115 and 201 to 206, the speed, charge conditioning capability and radiation tolerance were estimated in the same manner as in Example 1. Further, estimation of the high speed coatability thereof was carried out.

## (Estimation of High Speed Coatability)

The 16th layer in which the particle diameter of B-1 was set at 3  $\mu\text{m}$  was applied at a speed of 1 m/sec in accordance with the slide bead coating method and immediately dried. The number of cissings having occurred on the coating film surface was visually counted and assessed in terms of cission degree. The cission degree refers to the percentage of the number of cissings of each of the samples based on the number of cissings of the sample 110. The smaller the value of cission degree, the greater the cission inhibiting effect.

TABLE 4

| Sample | Electron-releasing compound | S(370 nm)/(420 nm) | Surfactant in 16th layer | Relative sensitivity<br>(See foot note) | Static-induced fog | Increment in fog due to radiation<br>(See foot note) |         |      |
|--------|-----------------------------|--------------------|--------------------------|-----------------------------------------|--------------------|------------------------------------------------------|---------|------|
|        |                             |                    |                          |                                         |                    | Cission characteristics                              | Remarks |      |
| 110    | Exemplified compound 7      | 0.22               | W-1                      | 150                                     | ◎                  | 87                                                   | 100     | Inv. |
| 201    | Exemplified compound 7      | 0.23               | FS-201                   | 152                                     | ◎                  | 84                                                   | 78      | Inv. |
| 202    | Exemplified compound 7      | 0.22               | FS-204                   | 151                                     | ◎                  | 86                                                   | 81      | Inv. |
| 203    | Exemplified compound 7      | 0.22               | FS-312                   | 151                                     | ◎                  | 85                                                   | 83      | Inv. |
| 115    | Exemplified compound 37     | 0.21               | W-1                      | 139                                     | ◎                  | 85                                                   | 114     | Inv. |
| 204    | Exemplified compound 37     | 0.20               | FS-201                   | 138                                     | ◎                  | 87                                                   | 65      | Inv. |
| 205    | Exemplified compound 37     | 0.22               | FS-204                   | 138                                     | ◎                  | 87                                                   | 66      | Inv. |
| 206    | Exemplified compound 37     | 0.22               | FS-312                   | 139                                     | ◎                  | 86                                                   | 64      | Inv. |

◎: No fog arose;

○: Very slight fog arose;

△: Slight fog arose;

×: Much fog arose.

(Note)

Relative speed and increment in fog due to radiation are indicated assuming those of Sample 101 as 100.

The results are listed in Table 4.

As apparent from Table 4, a striking effect in high speed coatability can be exerted, without detriment to the high

sensitivity, static tolerance and radiation tolerance, by the use of the surfactant according to the present invention.

## EXAMPLE 3

The support was prepared by the following procedure.

## 1) First Layer and Substratum:

Both major surfaces of a 90  $\mu\text{m}$  thick polyethylene naphthalate support were treated with glow discharge under such conditions that the treating ambient pressure was  $2.66 \times 10^3 \text{ Pa}$ , the  $\text{H}_2\text{O}$  partial pressure of ambient gas 75%, the discharge frequency 30 kHz, the output 2500 W, and the treating strength  $0.5 \text{ kV}\cdot\text{A}\cdot\text{min}/\text{m}^2$ . This support was coated, in a coating amount of 5  $\text{mL}/\text{m}^2$ , with a coating liquid of the following composition to provide the 1st layer in accordance with the bar coating method described in JP-B-58-4589.

|                                                                                                                                                                                                                                             |              |
|---------------------------------------------------------------------------------------------------------------------------------------------------------------------------------------------------------------------------------------------|--------------|
| Conductive fine grain dispersion<br>( $\text{SnO}_2/\text{Sb}_2\text{O}_5$ grain conc. 10% water<br>dispersion, secondary agglomerate of<br>0.005 $\mu\text{m}$ diam. primary grains which has an<br>av. grain size of 0.05 $\mu\text{m}$ ) | 50 pts. wt.  |
| Gelatin                                                                                                                                                                                                                                     | 0.5 pt. wt.  |
| Water                                                                                                                                                                                                                                       | 49 pts. wt.  |
| Polyglycerol polyglycidyl ether                                                                                                                                                                                                             | 0.16 pt. wt. |
| Polyoxyethylene sorbitan monolaurate<br>(polymn. degree 20)                                                                                                                                                                                 | 0.1 pt. wt.  |

The support furnished with the first coating layer was wound round a stainless steel core of 20 cm diameter and heated at 110° C. ( $T_g$  of PEN support: 119° C.) for 48 hr to thereby effect heat history annealing. The other side of the support opposite to the first layer was coated, in a coating

amount of 10  $\text{mL}/\text{m}^2$ , with a coating liquid of the following composition to provide a substratum for emulsion in accordance with the bar coating method.

|                                                       |                |
|-------------------------------------------------------|----------------|
| Gelatin                                               | 1.01 pts. wt.  |
| Salicylic acid                                        | 0.30 pt. wt.   |
| Resorcin                                              | 0.40 pt. wt.   |
| Polyoxyethylene nonylphenyl ether (polymn. degree 10) | 0.11 pt. wt.   |
| Water                                                 | 3.53 pts. wt.  |
| Methanol                                              | 84.57 pts. wt. |
| n-Propanol                                            | 10.08 pts. wt. |

Furthermore, the following second layer and third layer were superimposed in this sequence on the first layer by coating. Finally, multilayer coating of a color negative photosensitive material of the composition indicated below was performed on the opposite side. Thus, a transparent magnetic recording medium with silver halide emulsion layers was obtained.

2) Second Layer (Transparent Magnetic Recording Layer):

(i) Dispersion of Magnetic Substance:

1100 parts by weight of Co-coated  $\gamma$ -Fe<sub>2</sub>O<sub>3</sub> magnetic substance (average major axis length: 0.25  $\mu$ m,  $S_{BET}$ : 39  $m^2/g$ , Hc:  $65649 \times 10^4$  A/m, os: 77.1 Am<sup>2</sup>/kg, and or: 37.4 Am<sup>2</sup>/kg), 220 parts by weight of water and 165 parts by weight of silane coupling agent (3-(poly(polymerization degree: 10)oxyethyl)oxypropyltrimethoxysilane) were fed into an open kneader, and blended well for 3 hr. The resultant coarsely dispersed viscous liquid was dried at 70° C. round the clock to thereby remove water, and heated at 110° C. for 1 hr. Thus, surface treated magnetic grains were obtained.

Further, in accordance with the following recipe, a composition was prepared by blending by means of the open kneader once more for 4 hr:

|                                               |         |
|-----------------------------------------------|---------|
| Thus obtained surface treated magnetic grains | 855 g   |
| Diacetylcellulose                             | 25.3 g  |
| Methyl ethyl ketone                           | 136.3 g |
| Cyclohexanone                                 | 136.3 g |

Still further, in accordance with the following recipe, a composition was prepared by carrying out fine dispersion by means of a sand mill (1/4G sand mill) at 2000 rpm for 4 hr. Glass beads of 1 mm diameter were used as medium.

|                            |         |
|----------------------------|---------|
| Thus obtained blend liquid | 45 g    |
| Diacetylcellulose          | 23.7 g  |
| Methyl ethyl ketone        | 127.7 g |
| Cyclohexanone              | 127.7 g |

Moreover, in accordance with the following recipe, a magnetic substance containing intermediate liquid was prepared.

(ii) Preparation of Magnetic Substance Containing Intermediate Liquid:

|                                                                                                    |          |
|----------------------------------------------------------------------------------------------------|----------|
| Thus obtained fine dispersion of magnetic substance                                                | 674 g    |
| Diacetylcellulose solution (solid content 4.34%, solvent: methyl ethyl ketone/cyclohexanone = 1/1) | 24,280 g |
| Cyclohexanone                                                                                      | 46 g     |

These were mixed together and agitated by means of a disperser to thereby obtain a "magnetic substance containing intermediate liquid".

An  $\alpha$ -alumina abrasive dispersion of the present invention was produced in accordance with the following recipe.

(a) Preparation of Sumicorundum AA-1.5 (Average Primary Grain Diameter: 1.5  $\mu$ m, Specific Surface Area: 1.3 m<sup>2</sup>/g) Grain Dispersion

|                                                                                                   |          |
|---------------------------------------------------------------------------------------------------|----------|
| Sumicorundum AA-1.5                                                                               | 152 g    |
| Silane coupling agent KBM903 (produced by Shin-Etsu Silicone)                                     | 0.48 g   |
| Diacetylcellulose solution (solid content 4.5%, solvent: methyl ethyl ketone/cyclohexanone = 1/1) | 227.52 g |

In accordance with the above recipe, fine dispersion was carried out by means of a ceramic-coated sand mill (1/4G sand mill) at 800 rpm for 4 hr. Zirconia beads of 1 mm diameter were used as medium.

(b) Colloidal Silica Grain Dispersion (Fine Grains)

Use was made of "MEK-ST" produced by Nissan Chemical Industries, Ltd.

This is a dispersion of colloidal silica of 0.015  $\mu$ m average primary grain diameter in methyl ethyl ketone as a dispersion medium, wherein the solid content is 30%.

(iii) Preparation of a Coating Liquid for Second Layer:

|                                                                                                                                            |          |
|--------------------------------------------------------------------------------------------------------------------------------------------|----------|
| Thus obtained magnetic substance containing intermediate liquid                                                                            | 19,053 g |
| Diacetylcellulose solution (solid content 4.5%, solvent: methyl ethyl ketone/cyclohexanone = 1/1)                                          | 264 g    |
| Colloidal silica dispersion "MEK-ST" (dispersion b, solid content: 30%)                                                                    | 128 g    |
| AA-1.5 dispersion (dispersion a)                                                                                                           | 12 g     |
| Millionate MR-400 (produced by Nippon Polyurethane) diluent (solid content 20%, dilution solvent: methyl ethyl ketone/cyclohexanone = 1/1) | 203 g    |
| Methyl ethyl ketone                                                                                                                        | 170 g    |
| Cyclohexanone                                                                                                                              | 170 g    |

A coating liquid obtained by mixing and agitating these was applied in a coating amount of 29.3 mL/m<sup>2</sup> with the use of a wire bar. Drying was performed at 110° C. The thickness of magnetic layer after drying was 1.0  $\mu$ m.

3) Third Layer (Higher Fatty Acid Ester Sliding Agent Containing Layer)

(i) Preparation of Raw Dispersion of Sliding Agent

The following liquid A was heated at 100° C. to thereby effect dissolution, added to liquid B and dispersed by means of a high-pressure homogenizer, thereby obtaining a raw dispersion of sliding agent.

|                                                                     |               |
|---------------------------------------------------------------------|---------------|
| Liquid A:                                                           |               |
| Compd. of the formula: $C_6H_{13}CH(OH)(CH_2)_{10}COOC_{50}H_{101}$ | 399 pts. wt.  |
| Compound of the formula: $n-C_{50}H_{101}O(CH_2CH_2O)_{16}H$        | 171 pts. wt.  |
| Cyclohexanone                                                       | 830 pts. wt.  |
| Liquid B:                                                           |               |
| Cyclohexanone                                                       | 8600 pts. wt. |

93

(iii) Preparation of spherical inorganic grain dispersion  
Spherical inorganic grain dispersion (c1) was prepared in accordance with the following recipe.

|                                                                                                                           |                 |
|---------------------------------------------------------------------------------------------------------------------------|-----------------|
| Isopropyl alcohol                                                                                                         | 93.54 pts. wt.  |
| Silane coupling agent KBM903<br>(produced by Shin-Etsu Silicone)                                                          | 5.53 pts. wt.   |
| Compound 1-1: $(\text{CH}_3\text{O})_3\text{Si}-(\text{CH}_2)_3-\text{NH}_2$                                              |                 |
| W-5                                                                                                                       | 2.93 pts. wt.   |
| Seahostar KEP50 (amorphous spherical silica, av. grain size 0.5 $\mu\text{m}$ , produced by Nippon Shokubai Kagaku Kogyo) | 88.00 pts. wt.  |
| This composition was agitated for 10 min, and further the following was added:                                            |                 |
| Diacetone alcohol                                                                                                         | 252.93 pts. wt. |

The resultant liquid was dispersed by means of ultrasonic homogenizer "Sonifier 450 (manufactured by Branson)" for 3 hr while cooling with ice and stirring, thereby finishing spherical inorganic grain dispersion c1.

(iii) Preparation of Spherical Organic Polymer Grain Dispersion

Spherical organic polymer grain dispersion (c2) was prepared in accordance with the following recipe.

|                                                                                                                                  |              |
|----------------------------------------------------------------------------------------------------------------------------------|--------------|
| XC99-A8808 (produced by Toshiba Silicone Co., Ltd., spherical crosslinked polysiloxane grain, av. grain size 0.9 $\mu\text{m}$ ) | 60 pts. wt.  |
| Methyl ethyl ketone                                                                                                              | 120 pts. wt. |
| Cyclohexanone<br>(solid content 20%, solvent: methyl ethyl ketone/cyclohexanone = 1/1)                                           | 120 pts. wt. |

This mixture was dispersed by means of ultrasonic homogenizer "Sonifier 450 (manufactured by Branson)" for 2 hr while cooling with ice and stirring, thereby finishing spherical organic polymer grain dispersion c2.

(iv) Preparation of Coating Liquid for 3rd Layer

A coating liquid for 3rd layer was prepared by adding the following components to 542 g of the aforementioned raw dispersion of sliding agent:

|                                                                   |        |
|-------------------------------------------------------------------|--------|
| Diacetone alcohol                                                 | 5950 g |
| Cyclohexanone                                                     | 176 g  |
| Ethyl acetate                                                     | 1700 g |
| Above Seahostar KEP50 dispersion (c1)                             | 53.1 g |
| Above spherical organic polymer grain dispersion (c2)             | 300 g  |
| FC431 (produced by 3M, solid content 50%, solvent: ethyl acetate) | 2.65 g |
| BYK310 (produced by BYK ChemiJapan, solid content 25%)            | 5.3 g. |

The above third layer coating liquid was applied onto the second layer in a coating amount of 10.35 mL/m<sup>2</sup>, dried at 110° C. and further post-dried at 97° C. for 3 min.

4) Superimposing of Light-Sensitive Layer by Coating

Subsequently, multiple layers of compositions of the samples 101 to 115 were applied by coating onto the side opposite to obtained back layer, thereby obtaining color negative films.

The resultant samples were tested and evaluated in the same manner as in Example 1. The same excellent results as in Example 1 were obtained.

94

EXAMPLE 4

Samples whose spectral sensitivity in the ultraviolet region was changed were prepared by replacing (in equal silver amounts) the emulsions Em-H and Em-G in 9th layer, emulsion Em-F in 10th layer and emulsions Em-E and Em-G in 11th layer of the sample 101 with emulsions Em-H1, Em-G1, Em-F1, Em-E1 and Em-G1, respectively, or with emulsions Em-H2, Em-G2, Em-F2, Em-E2 and Em-G2, respectively, and by further changing the amounts of compounds UV-1 to -5 in 15th layer (first protective layer). Estimations of the obtained samples were performed in the same manner as in Example 1 except that density measurement was carried out through a green filter. When the amount of ultraviolet absorber used was small, the addition of electron-releasing compound, although a high sensitivity increasing effect was exerted, resulted in intensification of static-induced fog and radiation-induced fog. Photographic characteristics ensuring excellence in static tolerance and radiation tolerance while maintaining the advantage of sensitivity increase was realized through achieving of the spectral sensitivity distribution of the present invention by, while adding an electron-releasing compound, increasing the amount of ultraviolet absorber used.

EXAMPLE 5

Samples whose spectral sensitivity in the ultraviolet region was changed were prepared by replacing (in equal silver amounts) the emulsions Em-C and Em-D of 4th layer, emulsions Em-B and Em-C of 5th layer and emulsion Em-A of 6th layer of the sample 101 with emulsions Em-C1, Em-D1, Em-B1, Em-C1 and Em-A1, respectively, or with emulsions Em-C2, Em-D2, Em-B2, Em-C2 and Em-A2, respectively, and by further changing the amounts of compounds UV-1 to -5 of 15th layer (first protective layer). Estimations of the obtained samples were performed in the same manner as in Example 1 except that density measurement was carried out through a red filter. When the amount of ultraviolet absorber used was small, the addition of electron-releasing compound, although a high sensitivity increasing effect was exerted, resulted in intensification of static-induced fog and radiation-induced fog. Photographic characteristics ensuring excellence in static tolerance and radiation tolerance while maintaining the advantage of sensitivity increase was realized through achieving of the spectral sensitivity distribution of the present invention by, while adding an electron-releasing compound, increasing the amount of ultraviolet absorber used.

Additional advantages and modifications will readily occur to those skilled in the art. Therefore, the invention in its broader aspects is not limited to the specific details and representative embodiments shown and described herein. Accordingly, various modifications may be made without departing from the spirit or scope of the general inventive concept as defined by the appended claims and their equivalents.

60 What is claimed is:

1. A silver halide color photosensitive material comprising at least one each of a blue-sensitive layer, a green-sensitive layer, a red-sensitive layer and a non-light-sensitive layer on a support, wherein the silver halide color photosensitive material contains a compound selected from among the following type 1 and type 2 compounds, and

95

wherein the blue-sensitive layer meets the relationship of the following formula (I):

$$S_B(370 \text{ nm})/S_B(420 \text{ nm}) < 0.7 \quad (I)$$

wherein  $S_B(\lambda)$  represents a spectral sensitivity at a wavelength of  $\lambda$ ,

(type 1)

a compound capable of undergoing a one-electron oxidation to thereby form a one-electron oxidation product thereof, wherein the one-electron oxidation product is capable of releasing further one or more electrons accompanying a subsequent bond cleavage reaction, and

(type 2)

a compound capable of undergoing a one-electron oxidation to thereby form a one-electron oxidation product thereof, wherein the one-electron oxidation product is capable of releasing further one or more electrons accompanying a subsequent bond-forming reaction.

2. The silver halide color photosensitive material according to claim 1, wherein the silver halide color photosensitive material further contains at least one fluorinated surfactant selected from the group consisting of compounds represented by formula (A) and compounds represented by formula (B):

General formula (A)



wherein each of  $\text{R}^{B3}$ ,  $\text{R}^{B4}$  and  $\text{R}^{B5}$  independently represents a hydrogen atom or substituent, each of A and B

96

independently represents a fluorine atom or hydrogen atom, each of  $n^{B3}$  and  $n^{B4}$  is independently an integer of 4 to 8, each of  $\text{L}^{B1}$  and  $\text{L}^{B2}$  independently represents a substituted or unsubstituted alkylene group, substituted or unsubstituted alkyleneoxy group, or bivalent linking group composed of a combination thereof,  $m^B$  is 0 or 1, and M represents a cation;

General formula (B)



wherein  $\text{R}^{C1}$  represents a substituted or unsubstituted alkyl group, provided that the substituent does not include a fluorine atom,  $\text{R}^{CF}$  represents a perfluoroalkylene group, A represents a hydrogen atom or fluorine atom,  $\text{L}^{C1}$  represents a substituted or unsubstituted alkylene group, substituted or unsubstituted alkyleneoxy group, or bivalent linking group composed of a combination thereof, one of  $\text{Y}^{C1}$  and  $\text{Y}^{C2}$  represents a hydrogen atom while the other represents  $-\text{L}^{C2}-\text{SO}_3\text{M}$  wherein  $\text{L}^{C2}$  represents a single bond or substituted or unsubstituted alkylene group, and M represents a cation.

3. The silver halide color photosensitive material according to claim 1, wherein the compound selected from among type 1 and type 2 has an adsorptive group to silver halide in the molecule thereof.

\* \* \* \* \*